

[54] **DISPERSION OF SILVER HALIDE DEVELOPING AGENT WITH SURFACE ACTIVE POLYMERS OF MALEIC ACID HALF ESTERS**

3,518,088 6/1970 Dunn et al. .... 96/76 R  
3,589,902 6/1971 Himmelmann et al. .... 96/66 R  
3,647,437 3/1972 Land. .... 96/3  
3,765,897 10/1973 Nittel. .... 96/114.5  
3,785,824 1/1974 Fisch. .... 96/66.1

[75] Inventors: **Masami Miyakawa; Masakazu Yoneyama; Nobuo Yamamoto**, all of Minami-ashigara, Japan

*Primary Examiner*—David Klein  
*Assistant Examiner*—Richard L. Schilling  
*Attorney, Agent, or Firm*—Sughrue, Rothwell, Mion, Zinn & Macpeak

[73] Assignee: **Fuji Photo Film Co., Ltd.**, Minami-ashigara, Japan

[22] Filed: **July 26, 1974**

[21] Appl. No.: **492,312**

[30] **Foreign Application Priority Data**

July 26, 1973 Japan..... 48-84438

[52] **U.S. Cl.**..... **96/66 R**; 96/3; 96/29 D; 96/76 R; 96/77; 96/95; 96/97; 96/114.5

[51] **Int. Cl.<sup>2</sup>** .. **G03C 5/30**; G03C 1/48; G03C 1/40; G03C 1/10

[58] **Field of Search**..... 96/66 R, 77, 76 R, 97, 96/114.5, 29 D, 3, 95, 114.4

[56] **References Cited**

UNITED STATES PATENTS

2,322,027 6/1943 Jolley et al. .... 96/97  
3,121,011 2/1964 Haas et al. .... 96/3

[57] **ABSTRACT**

A dispersion comprising an hydrophilic organic colloid, fine droplets of silver halide developing agent dissolved in a substantially water-insoluble solvent, and a surface active polymer containing therein recurring units represented by the formula (I):



wherein R is a hydrocarbon chain or fluorine substituted hydrocarbon chain containing 4 to 22 carbon atoms, or an aryl group; n is 0 or an integer of 1 to 40; and M is a hydrogen atom or a cation.

**54 Claims, No Drawings**

**DISPERSION OF SILVER HALIDE DEVELOPING AGENT WITH SURFACE ACTIVE POLYMERS OF MALEIC ACID HALF ESTERS**

**BACKGROUND OF THE INVENTION**

**1. Field of the Invention**

The present invention relates to a dispersion of a silver halide developing agent in a hydrophilic organic colloid, which is contained in a color photographic element. The dispersion is applicable particularly to the diffusion transfer color process.

**2. Description of the Prior Art**

One of the diffusion transfer color processes is the dye developer process, which is described in British Pat. No. 804,971, U.S. Pat. Nos. 3,415,644, 3,415,645, 3,415,646, 3,594,164 and 3,594,165, and Japanese Patent Publication No. 16356/1971, etc. In this process, a photographic element comprising a silver halide emulsion layer and a layer containing a dye developer which is diffusible in an alkaline solution (a dye which acts to develop silver halide), is exposed to form a latent image in the silver halide and is processed with an alkaline composition which can permeate the silver halide emulsion layer and the layer containing the dye developer, whereby the latent image is developed with the dye developer which is diffused with the alkali and at the same time, an oxidation product of the dye developer is produced and is rendered essentially non-diffusible in the hydrophilic colloidal layer.

It is apparent that the non-diffusion of the oxidized dye developer is partially due to the reduced solubility thereof in the alkaline composition and that the diffusion of the oxidized dye developer in the hydrophilic colloidal layer is prevented by the hardening action of the oxidized dye developer on the hydrophilic colloid.

The unoxidized dye developer is partially or entirely transferred to an image receiving element overlaid thereon through diffusion, thereby providing a positive dye image.

Where an element is used which contains silver halide emulsion layers having different sensitivity and dye developers capable of providing color images corresponding to the color sensitivity of the silver halide emulsion layers, after exposure followed by processing with an alkaline composition, the remaining dye developer which is not consumed at the time of the development of the silver halide emulsions is transferred to a receiving element, whereby a multi-color positive image is obtained.

For instance, a dye former which provides a cyan transfer image is present in a red sensitive emulsion layer or in a colloidal layer adjacent the emulsion layer. A dye former which provides a magenta transfer image is present in a green sensitive emulsion layer or in a colloidal layer adjacent the emulsion layer. A dye former which provides a yellow transfer image is present in a blue sensitive layer or in a colloidal layer adjacent the emulsion layer. A photosensitive element comprising the above described red sensitive layer, green sensitive layer, and blue sensitive layer is exposed and treated with an alkaline composition, whereby a multi-color positive image is transferred to a receiving element overlaid on the photosensitive element. In this case, it is preferred that auxiliary developing agents are used to facilitate the development of the silver halide and the fixing of the dyes in the photosensitive element. The auxiliary developing agents are colorless, water-

insoluble, and soluble and diffusible in an alkaline solution through a hydrophilic organic layer such as gelatin.

It is necessary that the colloidal particles of the dye developer or the auxiliary developing agent be as small as possible and thus that the surface thereof be as large as possible. The reason is that the dissolution, diffusion and permeation of the dye developer or the auxiliary developing agent in the alkaline solution at the developing step is effected through the interface between the dispersed particles and the gelatin gel.

Mechanical techniques as well as surface chemical techniques are employed to prepare the above described fine particle dispersion. As the surface chemical techniques, surface active agents are generally used as an emulsifying agent. The emulsifying agent is effective in not only preparing fine particles, but providing storage stability for the particles for a long period of time. Preferably, the dispersion is stored after cool-setting or removing the solvent of the developing agent by evaporation or washing for the purpose of preventing the recombination of colloidal particles and preventing the crystal growth of the developing agent. With this procedure, however, it is difficult to store the dispersion for a long period of time while maintaining a fine particle size and without causing a crystallization of the developing agent. It is particularly difficult to eliminate the crystallization in the developing agent dispersion layer after the layer is coated and dried.

The dye developer should be non-diffusible and should not form coarse crystal grains in the photosensitive element prior to the alkaline solution processing and during the alkaline solution processing and it should be diffusible in the hydrophilic colloid. The introduction of various oleophilic substituents in the dye developer will render the dye developer easily soluble in a water-insoluble solvent for dispersion, but diffusion of the resulting dye developer is difficult at the processing stage. Thus, it is generally impossible to introduce a highly oleophilic substituent. In general, therefore, the dye developer has a low degree of dispersability in the water-insoluble solvent and coarse crystal grains tend to form in a dispersion thereof in an aqueous gelatin solution.

Thus, it is quite difficult to prepare an emulsion which is free from aggregation and crystallization with time, by emulsifying and dispersing the dye developer which is not suitable for emulsification and dispersion from a chemical structure standpoint, in a hydrophilic organic colloidal solution in the form of fine colloidal particles (the diameter of which desirably is below about 0.5 microns). It is very important to find effective emulsifying and dispersing agents. Where an emulsifying agent for an oil-soluble coupler, which is often used for conventional color photographic photosensitive element, is applied to the emulsification and dispersion of a dye developing agent, the crystallization and growth of the grains often occurs as is indicated in the Examples as described hereinafter.

In emulsifying and dispersing using a combination of gelatin and a surface active agent, difficult problems are caused by the foaming properties of the emulsifying agent, e.g., the emulsifying efficiency is lowered. Particularly, the coating of the emulsion and the photographic emulsion at the subsequent step becomes difficult. That is, a large amount of bubbles are incorporated in the liquid through vigorous stirring and the shearing force of an emulsifying machine is considerably reduced by the cushioning effect of the bubbles and

is not sufficiently transferred to the liquid droplets containing the dye developer and/or the auxiliary developing agent. As a result, the emulsifying efficiency is greatly reduced. Moreover, the fine air bubbles incorporated in the emulsion at the emulsifying stage often remain in the coating liquid, resulting in the formation of pin-holes when coated. In general, when the emulsifying agent used in emulsifying and dispersing the dye developer agent has a surface activity which is too high, such is not desirable in that the above mentioned crystallization and formation of air bubbles result. On the other hand, when the emulsifying agent has excellent emulsifying and dispersing capability, but has low surface activity and low spreadability, the coating of the emulsion becomes difficult.

Thus, the techniques to sufficiently finely disperse the dye developer, to prevent the dye developer from becoming coarse-grained, and to provide the dye developer with high reactivity and diffusibility with the alkaline solution for developing silver halide in the adjacent layer, are quite specific and conventionally used emulsifying and dispersing techniques can not be applied to achieve these results.

#### SUMMARY OF THE INVENTION

It is an object of the present invention to provide a dispersion wherein a compound capable of acting as a reductant for an exposed silver halide, such as a dye developer and/or an auxiliary developing agent (which developing agent or developing agents are herein referred to as a silver halide developing agent), is contained in a hydrophilic organic colloid in the form of fine colloidal particles without adversely affecting the photographic properties.

It is another object of the present invention to provide a dispersion wherein the silver halide developing agent emulsified and dispersed is prevented from aggregation and crystal separation with time.

It is a further object of the present invention to provide a dispersion suitable for providing an emulsion layer in which crystal separation of the dye developer is prevented.

These objects can be attained in a system comprising a hydrophilic organic colloid containing fine particles of a silver halide developing agent dissolved in a substantially water-insoluble solvent and at least one surface active polymer containing the recurring unit represented by the general formula (I):



wherein R is a hydrocarbon chain or fluorine substituted hydrocarbon chain containing 4 to 22 carbon atoms, or an aryl group; n is 0 or an integer of 1 to 40; and M is a hydrogen atom or a cation.

#### DETAILED DESCRIPTION OF THE INVENTION

In accordance with the present invention using the above described polymers, the dye developer and the auxiliary developing agent, the emulsification and dispersion of which have so far been difficult, can be effectively emulsified and dispersed, and an excellent dispersion can be obtained.

The hydrocarbon chain or fluorine substituted hydrocarbon chain can be a straight or branched chain, or

can contain unsaturated bonds provided that it contains 4 to 22 carbon atoms. Suitable examples of hydrocarbon chains having 4 to 22 carbon atoms include n-butyl, sec-butyl, iso-butyl, tert-butyl, n-amyl, iso-amyl, neopentyl, tert-amyl, n-hexyl, pinacolyl, n-heptyl, pentamethylethyl, n-octyl, iso-octyl, n-nonyl, n-decyl, n-dodecyl, n-tetradecyl, n-hexadecyl, n-pentadecyl, n-eicosyl, etc., suitable examples of fluorine substituted hydrocarbon chains, having 4 to 22 carbon atoms include 3,3,4,4-tetrafluorobutyl, dodecafluorononyl, tetracosafluorotridecyl, octacosafluoropentadecyl, perfluoroctyl, perfluorohaptadecyl, etc., and examples of hydrocarbon chains containing unsaturation include crotyl, 1-methyl-2-propenyl, 1-di-methyl-3-but enyl, 3-but enyl, 10-undecenyl, 1-methyl-2-but enyl, cis-9-octadecenyl, 4-pentenyl, 2,4-pentadienyl, 1-methyl-3-but enyl, 2,4-hexadienyl, 1-vinyl-2-but enyl, etc. Representative examples of aryl groups are unsubstituted aryl groups such as phenyl and naphthyl, and substituted aryl groups containing substituents such as alkyl, e.g., dodecyl; alkylamino, e.g., oleylamino; alkoxycarbonyl, e.g., octoxycarbonyl; acyloxy, e.g., octanoyloxy; acylamino, e.g., octanoylamino; alkylcarbamyl, e.g., octylcarbamoyl; and the like. These aryl groups suitably contain up to 22 carbon atoms, e.g., 6 to 22 carbon atoms.

Representative examples of M are hydrogen ion, and cations, e.g., alkali metal ions such as sodium ion, potassium ion and the like, ammonium ion, and trialkyl ammonium ion such as trimethyl ammonium ion, etc.

The surface active polymers containing the recurring unit represented by the above described formula include those copolymers produced from maleic anhydride or maleic acid half ester salts, and monomers copolymerizable therewith, such as ethylene, styrene, methyl vinyl ether, methyl methacrylate, ethyl acrylate, acrylonitrile, acrylamide, vinyl acetate, vinyl chloride, and the like. The polymer produced from maleic anhydride must be cleaved by alcohol decomposition. However, the present invention is not limited to the above described polymers only and all the polymers containing the above recurring unit can be used in the present invention. Polymers are suitable to achieve the objects of this invention as long as the amount of the repeating unit of the formula (I) is at least 10 percent by weight.

A preferred embodiment of these copolymers can be represented by the following general formulae (II) and (III).



wherein R, n and M are as defined above and the molar ratio of x to y ranges from 3:1 to 9:1. Copolymers of the general formula (II) above are particularly preferred.



Compound 15



These polymers as used in the present invention can be derived from commercially available copolymers. For instance, when an ethylene/maleic anhydride copolymer or a methyl vinyl ether/maleic anhydride copolymer is heated to about 100°C together with an ethylene oxide adduct of an alkylphenol or an aliphatic alcohol, the maleic anhydride unit is cleaved to provide the half ester thereof. An alkali salt derivative can be produced by dissolving the product prepared as described above in an aqueous alkali by heating. On the other hand, the copolymers can be easily produced in a conventional manner, e.g., as disclosed in U.S. Pat. Nos. 3,549,605; 3,448,708; and 3,525,620. The molecular weight of the copolymers is not limited and can range from about 250 to 100,000. Preferably the molecular weight of the copolymers ranges from about 1,000 to 20,000. The amount of the surface active polymer added varies depending on the kind of silver halide developing agent and the solvent, and the amount of the silver halide developing agent and solvent, and the amount can range up to about 200% by weight. Preferably it is in the range of about 0.5 to 50% by weight based on the weight of the silver halide developing agent. The surface active polymer can be used alone or in combination with surface active agents with anionic and nonionic surface active agents being preferred. Suitable surface active agents include the following examples.

## Aliphatic acid salts:

sodium myristate, sodium palmitate, sodium stearate, sodium oleate, sodium linoleate, sodium laurate, sodium caprate, potassium laurate, potassium stearate, etc.,

## Alkylsulfates:

sodium octadecylsulfate, sodium decylsulfate, sodium dodecylsulfate, sodium tetradecylsulfate, sodium hexadecylsulfate, potassium decylsulfate, potassium oleylsulfate, etc.,

## Alkylphosphates:

sodium octylphosphate, sodium dioctylphosphate, sodium nonylphosphate, sodium decylophosphate, potassium undecylphosphate, potassium dodecylphosphate, potassium pentadecylphosphate, etc.,

## Alkylsulfonates:

sodium dodecylsulfonate, sodium hexadecanesulfonate, sodium octadecanesulfonate, etc.,

## Alkyaryl sulfonates:

potassium octylbenzenesulfonate, sodium nonylbenzenesulfonate, sodium decylbenzenesulfonate, sodium undecylsulfonate, sodium dodecylbenzenesulfonate, sodium tridecylbenzenesulfonate, sodium dibutylnaphthalenesulfonate, sodium decylnaphthalenesulfonate, sodium octylnaphthalenesulfonate, potassium pentyl-naphthalenesulfonate, etc.,

Formaldehyde-condensates with alkynaphthalenesulfonates:

sodium formaldehyde-condensate with naphthalenesulfonate, sodium formaldehyde-condensate with butylnaphthalenesulfonate, etc.,

## Alkyldiphenylether sulfonates:

sodium nonyldiphenylether sulfonate, sodium decyl-diphenylether sulfonate, sodium dodecyl-diphenylether disulfonate, etc.

## Dialkylsulfosuccinates:

sodium dihexylsulfosuccinate, sodium dioctylsulfosuccinate, sodium dinonylsulfosuccinate, etc., Polyoxyethylene alkyl ethers and the sulfuric ester salts thereof:

10 polyoxyethylene lauryl ether, polyoxyethylene oleyl ether, sodium polyoxyethylene lauryl ether sulfate, sodium polyoxyethylene oleyl ether sulfate, polyoxyethylene dodecyl ether, polyoxyethylene tetradecyl ether, polyoxyethylene hexadecyl ether, polyoxyethylene octadecyl ether, etc.,

Polyoxyethylene alkylaryl ethers and the sulfuric ester salts thereof:

sodium polyoxyethylene nonylphenyl ether sulfate, polyoxyethylene nonylphenyl ether, sodium polyoxyethyl dibutylphenyl ether sulfate, etc.,

Polyoxyethylene alkyl esters and the sulfuric ester salts thereof:

20 polyoxethylene stearic acid ester, polyoxethylene palmitic acid ester, sodium polyoxethylene stearic acid ester sulfate, sodium polyoxethylene lauric acid ester sulfate, sodium polyoxethylene capric acid ester sulfate, sodium polyoxethylene myristic acid ester sulfate, etc.,

## Sorbitan alkyl esters:

30 sorbitan monolauric acid ester, sorbitan monopalmitic acid ester, sorbitan monostearic acid ester, sorbitan tristearic acid ester, sorbitan monooleic acid ester, sodium sorbitan trioleate, etc.,

## Polyoxyethylene sorbitan alkyl esters:

35 polyoxyethylene sorbitan monolauric acid ester, polyoxyethylene sorbitan monostearic acid ester, polyoxyethylene monooleic acid ester, polyoxyethylene sorbitan monopalmitic acid ester, polyoxyethylene trioleic acid ester, etc.,

## Others:

40 polyoxyethylene mannan monolauric acid ester, styrenemaleic acid half ester copolymer, etc.

The dye developers as used in the present invention are dye developers, which are described in U.S. Pat.

45 Nos. 2,983,605, 2,983,606, 2,992,106, 3,047,386, 3,076,808, 3,076,820, 3,077,402, 3,126,280, 3,131,061, 3,134,762, 3,134,765, 3,135,604, 3,135,604, 3,135,606, 3,135,734, 3,141,772, 3,142,565, 3,128,164, 3,230,082, 3,230,083, 3,239,339, 3,320,063, 3,453,107, 3,579,334, 3,482,972, and 3,563,739; Australian Pat. No. 220,279; German Pat. No. 1,036,640; British Pat. Nos. 804,971, 804,973, 804,974, and 804,975; Belgian Pat. Nos. 554,935 and 568,344; Canadian Pat. Nos. 579,038 and 577,021; French Pat. No. 1,168,292; etc.

55 The dye developers are characterized in that they are slightly soluble in water and non-diffusible under acidic and neutral conditions and they are diffusible under alkaline condition.

60 Representative examples of the dye developers include the following compounds.

1-Phenyl-3-N-n-hexylcarbamoyl-4-p-(2-hydroquinonyl-ethyl)-phenylazo-5-pyrazolone  
2-p-(2-Hydroquinonyl-ethyl)-phenylazo-4-isopropoxy-1-naphthol

- 1,4-bis[ $\beta$ -(Hydroquinonyl-isopropyl)amino]-5,8-dihydroxyanthraquinone  
 1-Phenyl-3-n-butyl-carbamoyl-4-[p-(2',5'-dihydroxyphenethyl)-phenylazo]-5-pyrazolone  
 1-Phenyl-3-N-n-hexylcarbamoyl-4-[p-(2',5'-dihydroxyphenethyl)-phenylazo]-5-pyrazolone  
 1-Phenyl-3-carbethoxy-4-[p-(2',5'-dihydroxyphenethyl)-phenylazo]-5-pyrazolone  
 2-[p-(2',5'-Dihydroxyphenethyl)phenylazo]-4-isopropoxy-1-naphthol  
 1-Phenyl-3-N-cyclohexylcarbamoyl-4-[p-(2',5'-dihydroxyphenethyl)-phenylazo]-5-pyrazolone  
 1-Phenyl-3-phenyl-4-[p-(2',5'-dihydroxyphenethyl)-phenylazo]-5-pyrazolone  
 1-Phenyl-3-amido-4-{4'-[p-(2",5"-dihydroxyphenethyl)-phenylazo]-2,5'-diethoxyphenylazo}-5-pyrazolone  
 1-Phenyl-3-N-cyclohexylcarbamoyl-4-[p-(2',5'-dihydroxyphenethyl)-phenylazo]-5-pyrazolone  
 1-Phenyl-3-phenyl-4-[p-(2',5'-dihydroxyphenethyl)-phenylazo]-5-pyrazolone  
 1-Phenyl-3-methyl-4-[p-(2',5'-dihydroxyphenethyl)-phenylazo]-5-pyrazolone  
 1-Phenyl-3-(N-n-heptyl)-carbamoyl-4-[p-( $\beta$ -hydroquinonylethyl)-phenylazo]-5-pyrazolone  
 1-(2'-Chlorophenyl)-3-(N-n-hexylcarbamoyl)-4-[p-( $\beta$ -hydroquinonylethyl)-phenylazo]-5-pyrazolone



- 2-[p-(2',5'-Dihydroxyphenethyl)-phenylazo]-4-methoxy-1-naphthol  
 2-[p-(2',5'-Dihydroxyphenethyl)phenylazo]-4-ethoxy-1-naphthol  
 2-[p-(2',5'-Dihydroxyphenethyl)-phenylazo]-4-n-propyl-1-naphthol



- 2-[p-(2',5'-Dihydroxyphenethyl)-phenylazo]-4-[1",4"-dioxahexyl]-1-naphthol  
 1,4-bis[ $\beta$ -(2',5'-Dihydroxyphenyl)-ethylamino]-anthraquinone  
 1-Chloro-4-[ $\beta$ -(2',5'-dihydroxyphenyl)-ethylamino]-anthraquinone  
 N-Monobenzol-1,4-bis[ $\beta$ -(3',4'-dihydroxyphenyl)-ethylamino]-anthraquinone  
 N-Monobenzol-1,4-bis[ $\beta$ -(2',5'-dihydroxyphenyl)-ethylamino]-anthraquinone  
 5,8-Dihydroxy-1,4-bis[ $\beta$ -hydroquinonyl- $\alpha$ -methyl]-ethylamino]-anthraquinone  
 1,4-bis(2',5'-Dihydroxyaniline)-anthraquinone  
 1,5-bis(2',5'-Dihydroxyaniline)-4,8-dihydroxy-antraquinone  
 1,4-bis[ $\beta$ -Hydroquinonyl- $\alpha$ -ethyl)ethylamino]-anthraquinone  
 5-Hydroxy-1,4-bis[ $\beta$ -hydroquinonyl- $\alpha$ -methyl)-ethylamino]-anthraquinone  
 1-( $\beta$ -Hydroxy- $\alpha$ -ethyl-ethylamino)-4-( $\beta$ -hydroquinonyl- $\alpha$ -methyl-ethylamino)-anthraquinone  
 1-(Butanol-2'-amino)-5,8-dihydroxy-4-hydroquinonyl-isopropylamino-antraquinone

- 1-(2'-Methylphenyl)-3-(N-n-hexylcarbamoyl)-4-[p-( $\beta$ -hydroquinonylethyl)-phenylazo]-5-pyrazolone  
 1-Acetoxy-2-[p-( $\beta$ -hydroquinoneethyl)-phenylazo]-4-methoxynaphthalene  
 4-Isobutoxy-2-[p-( $\beta$ -hydroquinoneethyl)-phenylazo]-1-naphthol  
 2-[4'-[p-(2",5"-Dihydroxyphenethyl)-phenylazo]- $\alpha$ -naphthylazo]-4-methoxy-1-naphthol  
 2-[4'-[p-(2",5"-Dihydroxyphenethyl)-phenylazo]- $\alpha$ -naphthylazo]-4-methoxy-1-naphthol  
 4-[p-(2',5'-Dihydroxyphenyl)phenylazo]-5-acetamido-1-naphthol  
 4-[p-(2',5'-Dihydroxyphenethyl)-phenylazo]-5-benzamido-1-naphthol  
 2-[p-(2',5'-Dihydroxyphenethyl)-phenylazo]-4-[p-(2',5'-Dihydroxy-4'-methylphenethyl)-phenylazo]-4-propoxy-1-naphthol  
 2-[p-(2',5'-Dihydroxyphenethyl)-phenylazo]-4-acetamido-1-naphthol



- 1,4-bis[ $\beta$ -(2',5'-Dihydroxyphenyl)-isopropylamino]-anthraquinone



1-Acetoxy-2-{p-[ $\beta$ -(hydroquinonyl)-ethyl]-phenylazo}-4-methoxy-naphthalene  
 1-Acetoxy-2-{p-[ $\beta$ -(hydroquinonyl)-ethyl]-phenylazo}-4-[(2'-ethoxy)-ethoxy]-naphthalene  
 1-Acetoxy-2-{p-[ $\beta$ -(hydroquinonyl)-ethyl]-phenylazo}-4-isopropoxynaphthalene



1-Acetoxy-2-{p-[ $\beta$ -(hydroquinonyl)-ethyl]-phenylazo}-4-(1',4'-dioxapentyl)-naphthalene

- 50  $\alpha$ -[p-(2-Hydroquinonylethyl)-phenylazo]- $\beta$ -(2'-furyl)- $\beta$ -acetoxy-acrylonitrile  
 $\alpha$ -[p-(2-Hydroquinonylethyl)-phenylazo]- $\beta$ -(2'-benzofuranyl)- $\beta$ -acetoxy-acrylonitrile  
 $\alpha$ -[m-(2-Hydroquinonylethyl)-phenylazo]- $\beta$ -(2'-benzofuranyl)- $\beta$ -acetoxy-acrylonitrile  
 $\alpha$ -[m-(Hydroquinonylmethyl)-phenylazo]- $\beta$ -(2'-benzofuranyl)- $\beta$ -acetoxy-acrylonitrile  
 55  $\alpha$ -[p-(2-Hydroquinonylethyl)-phenylazo]- $\beta$ -[2'-(5'-bromofuryl)]- $\beta$ -acetoxy-acrylonitrile  
 $\alpha$ -[p-(2-Hydroquinonylethyl)-phenylazo]- $\beta$ -[2'-(5'-methoxybenzofuranyl)]- $\beta$ -acetoxy-acrylonitrile  
 $\alpha$ -[p-(2-Hydroquinonylethyl)-phenylazo]- $\beta$ -[2'-(5'-bromobenzofuranyl)]- $\beta$ -acetoxy-acrylonitrile  
 $\alpha$ -[p-(2-Hydroquinonylethyl)-phenylazo]- $\beta$ -[2'-(3'-methylbenzofuranyl)]- $\beta$ -acetoxy-acrylonitrile  
 $\alpha$ -Phenylazo- $\beta$ -[2-(5'-hydroquinonylacetoamido)benzofuranyl]- $\beta$ -acetoxy-acrylonitrile  
 60  $\alpha$ -[p-(2-hydroquinonylethyl)-phenylazo]- $\beta$ -(2'-benzofuranyl)- $\beta$ -methoxyacetoxy-acrylonitrile  
 65  $\alpha$ -[p-(2-hydroquinonylethyl)-phenylazo]- $\beta$ -(2'-benzofuranyl)- $\beta$ -methoxyacetoxy-acrylonitrile



- $\alpha$ -[(2-Methyl-5-hydroquinonylmethyl)-phenylazo]- $\beta$ -(2'-benzofuryl)- $\beta$ -acetoxy-acrylonitrile  
 $\alpha$ -[(2-Acetoxy-5-hydroquinonylmethyl)-phenylazo]- $\beta$ -(2'-furyl)- $\beta$ -acetoxy-acrylonitrile  
 $\alpha$ -{[2-Acetoxy-5-(2'-hydroquinonylethyl)]-phenylazo}- $\beta$ -(2'-benzofuryl)- $\beta$ -acetoxy-acrylonitrile  
 $\alpha$ -[(2-Acetoxy-5-hydroquinonylmethyl)-phenylazo]- $\beta$ -(2'-(5'-bromofuryl))- $\beta$ -acetoxy-acrylonitrile  
 $\alpha$ -[(2-Acetoxy-5-hydroquinonylmethyl)-phenylazo]- $\beta$ -(2'-(5'-methoxybenzofuryl))- $\beta$ -acetoxy-acrylonitrile  
 $\alpha$ -[(2-Acetoxy-5-hydroquinonylmethyl)-phenylazo]- $\beta$ -(2'-(5'-bromobenzofuryl))- $\beta$ -acetoxy-acrylonitrile  
 $\alpha$ -[(2-Acetoxy-5-hydroquinonylmethyl)-phenylazo]- $\beta$ -(2'-(3'-methylbenzofuryl))- $\beta$ -acetoxy-acrylonitrile  
 $\alpha$ -(2-Acetoxyphenylazo)- $\beta$ -(2'-(5'-hydroquinonylacetamido)benzofuryl))- $\beta$ -acetoxy-acrylonitrile

- $\alpha$ -[(2-Acetoxy-5-hydroquinonylmethyl)-phenylazo]- $\beta$ -(2'-benzofuryl)- $\beta$ -acetoxy-acrylonitrile  
2-[m-(Hydroquinonylmethyl)phenylazo]-3-butyroloxy-5-methyl-benzothiophene  
2-[(2'-Chloro-5-hydroquinonylmethyl)phenylazo]-3-acetoxybenzothiophene  
2-[p-(2'-Hydroquinonylethyl)-phenylazo]-3-acetoxybenzothiophene  
2-[p-(2'-Hydroquinonylethyl)phenylazo]-3-acetoxy-5-chlorobenzothiophene  
2-[(2'-Acetoxy-5'-hydroquinonylmethyl)-phenylazo]-3-acetoxybenzothiophene  
2-[(2'-Methyl-5'-hydroquinonylmethyl)phenylazo]-3-acetoxybenzothiophene



- 2-[m-(Hydroquinonylmethyl)phenylazo]-3-acetoxybenzothiophene  
1,4-bis(2',5'-Dihydroxyaniline)-9,10-dihydroxyanthracene  
1,5-bis(2',5'-Dihydroxyaniline)-4,8,9,10-tetrahydroxyanthracene  
1,4-bis[ $\beta$ -(2',5'-Dihydroxyphenyl)-isopropylamino]-9,10-dihydroxyanthracene  
1,4-bis[ $\beta$ -(2',5'-Dihydroxyphenyl)-ethylamino]-9,10-di-hydroxyanthracene  
1-Chloro-4-[ $\beta$ -(2',5'-dihydroxyphenyl)-ethylamino]-9,10-dihydroxyanthracene  
1,4-bis[ $\gamma$ -(2',5'-Dihydroxyphenyl)propylamino]-5,8,9,10-tetrahydroxyanthracene  
1[ $\gamma$ -(2',5'-Dihydroxyphenyl)-propylamino]-4-( $\beta$ -hydroxyethylamino)-5,8,9,10-tetrahydroxyanthracene  
1-[ $\beta$ -(2',5'-Dihydroxyphenyl)-ethylamino]-4-( $\beta$ -hydroxyethylamino)-5,8,9,10-tetrahydroxyanthracene  
1-[ $\beta$ -(2',5'-Dihydroxyphenyl)-ethylamino]-5-( $\beta$ -hydroxyethylamino)-4,8,9,10-tetrahydroxyanthracene  
1,5-bis[ $\beta$ -(Hydroquinonyl- $\alpha$ -methyl)-ethylamino]-4,8,9,10-tetrahydroxyanthracene  
1-[ $\beta$ -(2',5'-Dihydroxyphenyl)ethylamino]-4-hexylamino-5,8,9,10-tetrahydroxyanthracene  
1,4-bis[ $\beta$ -(Hydroquinonyl- $\alpha$ -ethyl)ethylamino]-5,8,9,10-tetrahydroxyanthracene  
1,4-bis[ $\beta$ -(Hydroquinonyl- $\alpha$ -methyl)ethylamino]-5,8,9,10-tetrahydroxyanthracene  
1,4-bis[ $\beta$ -(Hydroquinonyl- $\alpha$ -methyl)ethylamino]-5,8,9,10-tetrahydroxyanthracene  
1,4-bis[ $\beta$ -(Hydroquinonyl- $\alpha$ -ethyl)ethylamino]-9,10-dihydroxyanthracene  
1-[ $\beta$ -Hydroxy- $\alpha$ -ethyl-ethylamino]-4-( $\beta$ -hydroquinonyl- $\alpha$ -methyl-ethylamino)-9,10-dihydroxyanthracene  
1-(Butanol-2'-amino)-4-( $\beta$ -hydroquinonyl-isopropylamino)-5,8,9,10-tetrahydroxyanthracene  
1,8-bis[ $\beta$ -(Hydroquinonyl- $\alpha$ -methyl)ethylamino]-4,5,9,10-tetrahydroxyanthracene  
N-Monobenzol-1,4-bis[ $\beta$ -(3',4'-dihydroxyphenyl)-ethylamino]-9,10-dihydroxyanthracene  
N-Monobenzol-1,4-bis[ $\beta$ -(2',5'-dihydroxyphenyl)-ethylamino]-9,10-dihydroxyanthracene  
1,4-Diamino-2-[ $\epsilon$ -( $\alpha$ -methyl-2',5'-dihydroxyhydrocinnamido)-pentoxy]-9,10-dihydroxyanthracene  
1,4-Diamino-2-[ $\epsilon$ -( $\alpha$ -ethyl-2',5'-dihydroxyhydrocinnamido)-pentoxy]-9,10-dihydroxyanthracene  
1,4-Diamino-2-[ $\epsilon$ -(2',5'-dihydroxyhydrocinnamido)-pentoxy]-9,10-dihydroxyanthracene

15



1,4-bis[( $\gamma$ -Hydroquinonyl- $\alpha$ -methyl)-  
propylamino]-5,8,9,10-tetrahydroxyanthracene  
1-(o-Carboxyphenyl)-3-phenyl-4-[p-(2',5'-tri-  
fluoroacetoxy- $\beta$ -phenylethyl)phenylazo]-5-  
hydroxypyrazole lactone



1-(o-Carboxyphenyl)-3-N-phenylcarbamoyl-4-[p-  
( $\beta$ -hydroquinonylethyl)phenylazo]-5-hydrox-  
ypyrazole lactone  
 $\alpha$ {[2-Butyroyloxy-5-(2',5'-butyroyloxy-phenylmethyl)]-phenylazo}- $\beta$ -(2'-benzofuranyl)- $\beta$ -  
butyroyloxyacrylonitrile  
2-[m-(2',5'-Butyroyloxy-phenylmethyl)phenylazo]-  
3-butyroyloxybenzothiophene  
 $\alpha$ -[p-(2,5-Butyroyloxy- $\beta$ -phenylethyl)-phenylazo]- $\beta$ -  
(2'-benzofuranyl)- $\beta$ -butyroyloxy-acetonitrile

16

droquinone, 2-dimethylaminomethyltoluhydroquinone, 2-cyclohexylhydroquinone, sec-butylhydroquinone, 2,5-dichlorohydroquinone, 2,5-diisopropylhydroquinone, 2,5-diiodohydroquinone, 3-chlorotoluhydroquinone, tetrachlorohydroquinone, 2,5-diphenylhydroquinone, 2,5-diresorcylihydroquinone, 2,5-diocetylhydroquinone, dodecylhydroquinone, 4-methoxycatechol, 4-isopropoxycatechol, 3-isopropylcatechol, 4-phenylcatechol, 3,6-dimethylcatechol, 1,2-dihydroxy-5,8-methano-5,6,7,9-tetrahydronaphthalene, etc.

These silver halide developing agents are generally dissolved in a high boiling solvent (e.g., above 150°C) and, if desired, an auxiliary solvent, and dispersed in an about 1 to 20% by weight, preferably about 10% by weight, aqueous solution of a hydrophilic organic colloid such as gelatin, in the form of fine colloidal particles, having a particle size of less than about 1  $\mu$ , preferably less than 0.5  $\mu$ . With the high molecular weight surfactant of this invention a particle size of about 0.3  $\mu$  can be used.

In addition to the gelatin described above, the following can be used as the hydrophilic organic colloid: phthalated gelatin, polyvinyl alcohol, polyvinyl pyrrolidone, polyacrylamide, sodium polyacrylate, polyvinyl-2-methylidazole, acrylamide/1-vinyl-2-methylimidazole copolymers, acrylamide/imidazole copolymers, acrylamide/1-vinyl-2-methylimidazole/acrylic acid copolymers, nitrocarboxymethylcellulose, N-vinylpyrrolidone-acrylic acid copolymers, N-vinylpyrrolidone-acrylic acid-methyl acrylate copolymers, vinylphthalimide-acrylic acid copolymers, cellulose acetate hydrogen phthalate, poly-N-methylmethacrylamide, dimethylaminoethylmethacrylate-acrylic acid copolymers, dimethylaminoethylmethacrylate-acrylic acid-butyl acrylate copolymers, N,N-diethylacrylamide-acrylamide copolymers, poly-N-methylacrylamide copolymers, N-methylacrylamide-N-hydroxymethylacrylamide copolymers, poly-N-ethylacrylamide, methylvinylketoneacrylamide copolymers, N-vinylpyrrolidone-methacrolein copolymers, and the like. If desired, they can be used in combination with each other. Furthermore, they can be used in combination with



2-[p-(2',5'-Ethoxyxaloxoxyphenethyl)phenylazo]-  
4-methoxy-1-naphthol

Suitable auxiliary developing agents are described in British Pat. No. 1,243,539, U.S. Pat. No. 3,253,915, Belgian Pat. No. 722,298, French Pat. No. 1,599,790, Japanese Pat. Publication Nos. 29130/1964 and 13837/1968, etc. Representative examples of auxiliary developing agents are phenylhydroquinone, 2-hydroxyphenylhydroquinone, phenoxyhydroquinone, 4-methylphenylhydroquinone, 1,4-dihydroxynaphthalene, 2-(4-aminophenethyl)-5-bromohydroquinone, 2-(4-aminophenethyl)-5-methylhydroquinone, 4-aminophenethylhydroquinone, 2,5-dimethoxyhydroquinone, 2,5-dibutoxyhydroquinone, m-xylohydroquinone, bromohydroquinone, 3,6-dichlorohydro-

synthetic polymers such as cellulose acetate and the like. The high boiling solvent is an organic solvent which is used for dispersing the silver halide developing agent in the hydrophilic organic colloid such as gelatin and the like and has a low molecular weight, is capable of easily dissolving the silver halide developing agent, is substantially water-insoluble and preferably has a boiling point higher than about 150°C. The high boiling solvent is normally a liquid or a low melting solid at room temperature.

As the high boiling solvent, the following can be used: phosphoric acid esters such as triethyl phosphate, tri-n-butyl phosphate, triphenyl phosphate, tricresyl phosphate, tri-p-tert-butylphenyl phosphate, tri-2-ethylhexyl phosphate, and the like; phthalic acid esters

such as methyl phthalate, ethyl phthalate, n-butyl phthalate, 2-ethylbutyl phthalate, n-propyl phthalate, n-amyl phthalate, isoamyl phthalate, n-octyl phthalate,  $\beta$ -methoxyethyl phthalate, ditetrahydrofurfuryl phthalate and the like; aliphatic dibasic acid esters such as ditetrahydrofurfuryladipate, n-octyladipate, 2-ethylhexyladipate, n-hexyladipate, 2-ethylbutylacetate, butylsebacate, ditetrahydrofurfurlysuccinate, dibutoxyethylsuccinate, and the like; aliphatic monobasic acid esters such as oleic acid butyl ester, oleic acid tetrahydrofurfuryl ester, o-methoxyphenyl acetate, stearic acid butyl ester and the like; other esters such as triethyl citrate, acetyltriethyl citrate, triethyleneglycol di-2-ethyl hexoate, acetylricinol acid methyl ester, acetylricinol acid methoxyethyl ester,  $\gamma$ -acetoxybutylacetyl succinate, tetrahydrofurfuryl benzoate, and the like; amides and imides such as diethyl lauryl amide, dibutyl lauryl amide, tetraethyl phthalamide, N-n-butyl acetanilide, N-methyl-p-methyl acetanilide; N-n-amyl succinimide, N-n-amyl phthalimide, lauoyl piperidine, and the like; alcohols such as 4-methyl-2-pentanol, furfuryl alcohol, methyl isobutyl carbinol, 2,4-di-n-amyl phenol, and the like; ethers such as ethyleneglycol monobenzyl ether; and ketones such as ethyl-N, N-din-butylcarbamate, 2-methyl cyclohexanone, 3-methyl cyclohexanone, 4-methyl cyclohexanone, and the like, etc.

The auxiliary solvent is effective in that when used in combination with the high boiling solvent, the solubility of the dye developer and the auxiliary developing agent is increased and the grain size of the dispersion is reduced. The auxiliary solvent can be removed from the dispersion containing the high boiling solvent by air-drying or washing.

Representative examples of auxiliary solvents are esters such as  $\beta$ -ethoxyethyl acetate,  $\beta$ -butoxy- $\beta$ -ethoxyethyl acetate, tetrahydrofurfuryl adipate, ethyleneglycol monoacetate, methoxy triglycol acetate, ethyleneglycol monomethyl ether acetate, methyl acetate, ethyl acetate, propyl acetate, butyl acetate, isopropyl acetate, ethyl propionate, and the like; alcohols such as diacetone alcohol, ethylene glycol, diethylene glycol, dipropylene alcohol, sec-butyl alcohol, benzyl alcohol and the like; ketones such as methyl isobutyl ketone, methyl isopropyl ketone, acetonylacetone, cyclohexanone, 2-methylcyclohexanone, 3-methylcyclohexanone, 4-methylcyclohexanone, and the like; ethers such as diethylene glycol monobutyl ether, ethylene glycol monobutyl ether, diethylene glycol monoethyl ether, ethylene glycol monomethyl ether and the like; carbon tetrachloride and chloroform; etc.

The ratio of the silver halide developing agent to the binder is preferably in the range of about 2:1 to 1:2.

The dispersion of the present invention can contain, if desired, other additives.

For example, by adding an oleophilic polymer to the oil phase of the dispersion, the stability of the dispersion can be increased. Suitable examples thereof include polyvinyl acetate, polyvinyl butyral, polyvinyl chloride, polyvinyl propionate, polymethyl acrylate, polyethyl acrylate, polybutyl acrylate, polypropyl acry-

late, polymethylmethacrylate, polyethylmethacrylate, polybutylmethacrylate, polypropylmethacrylate, etc. In addition by adding a viscosity increasing agent, the stability of the dispersion can be increased. Representative examples thereof include polyacrylamide, cellulose nitrate, poly-p-sulfostyrene potassium salt, etc. Further, after the dispersion is coated, a hardening agent such as formaldehyde, mucochloric acid, 2-hydroxyl-4,6-dichloro-s-triazine sodium salt, etc., can be added to harden the coated layer.

The silver halide developing agent of the present invention is rendered free from the separation of the silver halide developing agent and coarse-graining of the fine liquid particles of the water-insoluble solvent in which the silver halide developing agent is contained, for a long period of time, and thus it is quite stable.

The dispersion of the present invention can be employed in the photographic elements disclosed in U.S. Pat. Nos. 2,983,606, 3,415,644, 3,415,645, 3,415,646, 3,594,164, and 3,594,165 and in the photographic materials as disclosed in U.S. Pat. Nos. 2,983,606, 3,345,163, 3,188,209 and 3,316,090.

The present invention will be described in greater detail by reference to the following examples. Unless otherwise indicated, all parts, percents, ratios, and the like are by weight.

#### EXAMPLE 1

To a mixture of 15 ml of N,N-diethyl lauryl amide and 22 ml of cyclohexanone was added 10 g of yellow dye developer: 1-phenyl-3-N-n-hexylcarbamoyl-4-p-(2-hydroquinonylethyl)phenylazo-5-pyrazolone. To the resulting solution, a 20% cyclohexanone solution of Compound 2 having an average molecular weight of about 4000 (in the amounts shown in Table 1) as the emulsifying agent and 2 ml of a 20% methanol solution of Span 20 (sorbitan monolauric acid ester produced by Atlas Powder Co.) were added and completely dissolved in the vicinity of about 80°C.

The solution so prepared was added to 120 g of a 10% aqueous solution of gelatin at about 80°C and stirred moderately. The resulting solution was dispersed with a colloid mill. The dispersion so prepared was cool-set and stored. The average grain size was about 0.3 to 0.4  $\mu$ .

The emulsion was coated on a gelatin undercoated cellulose triacetate base in a thickness of about 3  $\mu$  and on the resulting layer a gelatin aqueous solution having the following composition was coated to provide a dry thickness of about 1  $\mu$ .

|                                                              |        |
|--------------------------------------------------------------|--------|
| 10% Gelatin Aqueous Solution                                 | 40 g   |
| Water                                                        | 160 ml |
| 5% Polyoxyethylenesorbitan Monolauryl Ester Aqueous Solution | 8 ml   |
| 1% Mucochloric Acid Aqueous Solution                         | 1 ml   |

The sample so prepared was stored under the conditions of 50°C and 80% RH and the days until crystals of the dye developer separated were measured.

The results obtained are shown in Table 1.

Table 1

| Amount of Compound 2 | Days until Crystals of the Yellow Dye Developer Separated |
|----------------------|-----------------------------------------------------------|
| (grams)              | (days)                                                    |
| 0.4                  | 2-3                                                       |
| 0.8                  | More than 10                                              |
| 1.2                  | More than 10                                              |

## EXAMPLE 2

The procedure of Example 1 was repeated using magenta dye developer: 2-p-(2-hydroquinonylethyl)-phenylazo-4-isopropoxy-1-naphthol.

The results obtained are shown in Table 2.

Table 2

| Amount of Compound 2<br>(grams) | Days until Crystals of the Magenta<br>Dye Developer Separated<br>(days) |
|---------------------------------|-------------------------------------------------------------------------|
| 0.4                             | 2-3                                                                     |
| 0.8                             | 3-4                                                                     |
| 1.2                             | More than 10                                                            |

## EXAMPLE 3

The procedure of Example 1 was repeated using cyan dye developer: 1,4-bis  $\beta$ -(hydroquinonylpropyl)amino-5,8-dihydroxyanthraquinone.

The results obtained are shown in Table 3.

Table 3

| Amount of Compound 2<br>(grams) | Days until Crystals of the Cyan Dye<br>Developer Separated<br>(days) |
|---------------------------------|----------------------------------------------------------------------|
| 0.4                             | 1                                                                    |
| 0.8                             | 2                                                                    |
| 1.2                             | 2-3                                                                  |

## EXAMPLE 4

The procedure of Example 1 was repeated using magenta dye developer: 1-acetoxy-2-p-(2-hydroquinonylethyl)-phenylazo-4-isopropoxy-naphthalene.

The results are shown in Table 4.

Table 4

| Amount of Compound 2<br>(grams) | Days until Crystals of the Magenta<br>Dye Developer Separated<br>(days) |
|---------------------------------|-------------------------------------------------------------------------|
| 0.4                             | 3                                                                       |
| 0.8                             | More than 10                                                            |
| 1.2                             | More than 10                                                            |

## EXAMPLE 5

The procedure of Example 2 was repeated except

Table 5

| Amount of Compound 14<br>(grams) | Days until Crystals of the Magenta<br>Dye Developer Separated<br>(days) |
|----------------------------------|-------------------------------------------------------------------------|
| 0.4                              | 1                                                                       |
| 0.8                              | 2                                                                       |
| 1.2                              | 5                                                                       |

## EXAMPLE 6

10 g of magenta dye developer: 2-p-(2-hydroquinonylethyl)-phenylazo-4-isopropoxy-1-naphthol was added to 60 ml of 2-methylcyclohexanone. To the resulting solution, 5 g of polyvinyl hydrogen phthalate, 5 g of Compound 2 as the emulsifying agent, and 2 ml of a 20% methanol solution of Span 20 were added and dissolved in the vicinity of 80°C.

10 The resulting solution was added to 160 g of a 10% gelatin aqueous solution at about 80°C and stirred moderately. The solution was further dispersed using a colloid mill.

15 The dispersion was cool-set and stored. The resulting emulsion was coated on a gelatin subbed cellulose triacetate base in a thickness of about 3  $\mu$  and gelatin was coated on the layer as prepared above in a thickness of 1  $\mu$ .

20 The resulting sample was stored under the conditions of 50°C and 80% RH and the days until Crystal of the dye developer separated, were measured. The crystals of the dye developer did not separate for more than 10 days.

## COMPARISON EXAMPLE 1

The procedure of Example 2 was repeated except that Aerogel OT (bis-(2-ethylhexyl)sulfosuccinic acid sodium salt produced by American Cyanamid Co.) was used as the emulsifying agent and as magenta dye developer; 2-p-(2-hydroquinonylethyl)-phenylazo-4-isopropoxy-1-naphthol, was used.

25 The results obtained are shown in Table 6.

Table 6

| Amount of Aerosol OT<br>(grams) | Days until Crystals of the Magenta<br>Dye Developer Separated<br>(days) |
|---------------------------------|-------------------------------------------------------------------------|
| 0.4                             | Within 1                                                                |
| 0.8                             | Within 1                                                                |
| 1.2                             | Within 1                                                                |

## COMPARISON EXAMPLE 2

The procedure of Example 2 was repeated except that p-nonylphenoxypropylsulfonic acid sodium salt was used as the emulsifying agent and dispersed in a 10% gelatin aqueous solution and that magenta dye developer; 2-p-(2-hydroquinonylethyl)-phenylazo-4-isopropoxy-1-naphthol, was used.

45 The results obtained are shown in Table 7.

Table 7

| Amount of p-Nonylphenoxypropyl<br>Sulfonic Acid Sodium Salt<br>(grams) | Days until Crystals of the<br>Magenta Dye Developer Separated<br>(days) |
|------------------------------------------------------------------------|-------------------------------------------------------------------------|
| 0.4                                                                    | Within 1                                                                |
| 0.8                                                                    | Within 1                                                                |
| 1.2                                                                    | Within 1                                                                |

## COMPARISON EXAMPLE 3

50 The procedure of Example 4 was repeated using Aerogel OT as the emulsifying agent and magenta dye developer; 1-acetoxy-2-[p-(2-hydroquinonyethyl)-phenylazo]-4-isopropoxy-naphthalene.

The results obtained are shown in Table 8.

Table 8

| Amount of Aerosol OT<br>(grams) | Days until Crystals of the Magenta<br>Dye Developer Separated<br>(days) |
|---------------------------------|-------------------------------------------------------------------------|
| 0.4                             | Within 1                                                                |
| 0.8                             | Within 1                                                                |
| 1.2                             | Within 1                                                                |

that Compound 14 having an average molecular weight of about 3000 was used as the emulsifying agent and as the magenta dye developer: 2-p-(2-hydroquinonylethyl)-phenylazo-4-isopropoxy-1-naphthol was used.

The results obtained are shown in Table 5.

Table 5

| Amount of Compound 14<br>(grams) | Days until Crystals of the Magenta<br>Dye Developer Separated<br>(days) |
|----------------------------------|-------------------------------------------------------------------------|
| 0.4                              | 1                                                                       |
| 0.8                              | 2                                                                       |
| 1.2                              | 5                                                                       |

By comparing Examples 1 to 6 with Comparison Examples 1 to 3, it can be seen that the polymers of the present invention are quite effective in preventing the separation of crystals of the dye developer.

While the invention has been described in detail and with reference to specific embodiments thereof, it will be apparent to one skilled in the art that various changes and modifications can be made therein without departing from the spirit and scope thereof.

What is claimed is:

1. A silver halide developing agent dispersion which comprises a hydrophilic organic colloid having dispersed therein fine droplets of a silver halide developing agent dissolved in a substantially water-insoluble solvent, and at least one surface active polymer selected from the group consisting of the compounds represented by the following formulae (II) and (III):



and



wherein R is a hydrocarbon chain or a fluorine substituted hydrocarbon chain containing 4 to 22 carbon atoms or an aryl group, n is O or an integer of 1 to 40, and M is a hydrogen atom or a cation; and wherein the molar ratio of x to y ranges from 3:1 to 9:1.

2. The silver halide developing agent dispersion according to claim 1, wherein the surface active polymer has the general formula



wherein R, n, M, x and y are as defined in claim 2.

3. The silver halide developing agent dispersion according to claim 1, wherein the amount of the surface active polymer ranges from about 0.5 to 50% by weight based on the silver halide developing agent.

4. The silver halide developing agent dispersion according to claim 1, wherein the silver halide developing agent comprises at least one dye developer.

5. The silver halide developing agent dispersion according to claim 1, wherein the silver halide developing agent comprises at least one dye developer and at least one auxiliary developing agent.

6. The silver halide developing agent dispersion according to claim 1, wherein a solution of the silver halide developing agent in a high boiling solvent is dispersed in about 1 to 20% by weight aqueous solution of the hydrophilic organic colloid.

7. The silver halide developing agent dispersion according to claim 1, wherein the hydrophilic organic colloid is gelatin.

8. The silver halide developing agent dispersion according to claim 1, wherein the surface active polymer is selected from the group consisting of compounds represented by the following formulae:



wherein the molar ratio of x to y ranges from 3:1 to 9:1.

9. The silver halide developing agent dispersion according to claim 1, wherein the surface active polymer has a molecular weight from about 250 to about 100,000.

10. The silver halide developing agent dispersion according to claim 1, wherein the surface active polymer has a molecular weight from about 1,000 to 20,000.

11. The silver halide developing agent dispersion according to claim 2, wherein the surface active polymer is selected from the group consisting of compounds represented by the following formulae:



wherein the molar ratio of  $x$  to  $y$  ranges from 3:1 to 9:1.

12. The silver halide developing agent dispersion according to claim 2, wherein the surface active polymer has a molecular weight from about 250 to 100,000.

13. The silver halide developing agent dispersion according to claim 2, wherein the surface active polymer has a molecular weight from about 1,000 to 20,000.

14. The silver halide developing agent dispersion according to claim 1, wherein the dispersion further contains an anionic or nonionic surface active agent.

15. The silver halide developing agent dispersion according to claim 14, wherein the surface active agent is selected from the group consisting of aliphatic acid salts, alkylsulfates, alkylphosphates, alkyl-sulfonates, alkylarylsulfonates, formaldehyde-condensates with alkyl-naphthalenesulfonates, alkylidiphenyl-ether sulfonates, dialkylsulfosuccinates, polyoxyethylene, alkyl ethers and the sulfuric ester salts thereof, poly-oxyethylene alkyl ethers and the sulfuric ester salts thereof, poly-oxyethylene alkyl esters and the sulfuric ester salts thereof, sorbitan alkyl esters, polyoxyethylene sorbitan alkyl esters, polyoxyethylene manitan monolauric acid ester and styrene-maleic acid half ester copolymer.

16. The silver halide developing agent dispersion according to claim 14 wherein the surface active agent is selected from the group consisting of sodium myris-

tate, sodium palmitate, sodium stearate, sodium oleate, sodium linoleate, sodium laurate, sodium caprate, potassium laurate, potassium stearate, sodium octadecylsulfate, sodium decylsulfate, sodium dodecylsulfate, sodium tetradecylsulfate, sodium hexadecylsulfate, potassium decylsulfate, potassium oleylsulfate, sodium octylphosphate, sodium dioctylphosphate, sodium nonylphosphate, sodium decylphosphate, potassium undecylphosphate, potassium dodecylphosphate, potassium pentadecylphosphate, sodium dodecylsulfonate, sodium hexadecanesulfonate, sodium octadecanesulfonate, potassium octylbenzenesulfonate, sodium nonylbenzenesulfonate, sodium decylbenzenesulfonate, sodium undecylsulfonate, sodium dodecylbenzenesulfonate, sodium tridecylbenzenesulfonate, sodium dibutylnaphthalenesulfonate, sodium decylnaphthalenesulfonate, sodium octylnaphthalenesulfonate, potassium pentylnaphthalenesulfonate, sodium formaldehyde-condensate with naphthalenesulfonate, sodium formaldehyde-condensate with butyl-naphthalensulfonate, sodium nonyldiphenylether sulfonate, sodium decyldiphenylether sulfonate, sodium dodecyldiphenylether disulfonate, sodium dihexylsulfosuccinate, sodium dioctylsulfosuccinate, sodium dinonylsulfosuccinate, polyoxyethylene lauryl ether, polyoxyethylene oleyl ether, sodium polyoxyethylene lauryl ether sulfate, sodium polyoxyethylene oleyl ether sulfate, polyoxyethylene dodecyl ether, polyoxyethylene tetradecyl ether, polyoxyethylene hexadecyl ether, polyoxyethylene octadecyl ether, sodium polyoxyethylene nonylphenyl ether sulfate, polyoxyethylene nonylphenyl ether, sodium polyoxyethylene dibutylphenyl ether sulfate, polyoxyethylene stearic acid ester, polyoxyethylene palmitic acid ester, sodium polyoxyethylene stearic acid ester sulfate, sodium polyoxyethylene lauric acid ester sulfate, sodium polyoxyethylene capric acid ester sulfate, sodium polyoxyethylene myristic acid ester sulfate, sorbitan monostearic acid ester, sorbitan tristearic acid ester, sorbitan monooleic acid ester, sodium sorbitan trioleate, polyoxyethylene sorbitan monolauric acid ester, polyoxyethylene sorbitan monostearic acid ester, polyoxyethylene monooleic acid ester, polyoxyethylene sorbitan monopalmitic acid ester, poly-oxyethylene trioleic acid ester, polyoxyethylene manitan monolauric acid ester and styrene-maleic acid half ester copolymer.

17. The silver halide developing agent dispersion according to claim 4, wherein the dye developer is selected from the group consisting of 1-Phenyl-3-N-n-hexylcarbamoyl-4-p-(2-hydroquinonyl-ethyl)-phenylazo-5-pyrazolone, 2-p-(2-Hydroquinonyl-ethyl)-phenylazo-4-isopropoxy-1-naphthol, 1,4-bis[ $\beta$ ]-Hydroquinonyl-isopropyl)amino]-5,8-dihydroxy-anthraquinone, 1-Phenyl-3-n-butyl-carbamoyl-4-[p-(2', 5'-dihydroxyphenethyl)-phenylzao]-5-pyrazolone, 1-Phenyl-3-N-n-hexyl-carbamoyl-4-[p-(2', 5',-dihydroxyphenethyl)-phenylzao]-5-pyrazolone, 2, [p-(2', 5'-Dihydroxyphenethyl)phenylzao]-4-isopropoxy-1-naphthol, 1-Phenyl-3-N-cyclohexylcarbamoyl-4-[p-(2', 5'-dihydroxy-phenethyl)-phenylzao]-5-pyrazolone, 1-Phenyl-3-amido-4 { 4'[p-2', 5''-dihydroxy-phenethyl)-phenylzao] -2',5'-diethoxyphenylzao -5- } pyrazolone, 1-Phenyl-3-N-cyclohexylcarbamoyl-4-[p-(2', 5'-dihydroxy-phenethyl)-phenylzao]-5-pyrazolone, 1-Phenyl-3-phenyl-4-[p-(2', 5'-dihydroxyphenethyl)-phenylzao]-5-pyrazolone, 1-Phenyl-3-methyl-4-[p-1', 5'-dihydroxyphenethyl)-phenylzao]-5-pyrazolone, 1-Phenyl-3-(N-n-heptyl)carbamoyl-4-[p-( $\beta$ -

hydroquinonyl ethyl)-phenylazo]-5-pyrazolone, 1 -(2'-Chlorophenyl)-3-(N-n-hexylcarbamoyl)-4-[p-( $\beta$ -hydroquinonyl ethyl)-phenylazo]-5-pyrazolone,



1-(2'-Methylphenyl)-3-(N-n-hexylcarbamoyl)-4-[p-( $\beta$ -hydroquinonylethyl)-phenylazo]-5-pyrazolone, 1-Acetoxy-2-[p-( $\beta$ -hydroquinoneethyl)-phenylazo]-4-methoxy-naphthalene, 4-Isobutoxy-2-[p-( $\beta$ -hydroquinoneethyl)-phenylazo]-1-naphthol, 2 { 4'-[p-(2'',5''-Dihydroxyphenethyl)-phenylazo]- $\alpha$ -naphthyl-azo}-4-methoxyl-1-naphthol, 2-[p-(2', 5'-Dihydroxy-4'-methylphenethyl)-phenylazo]-4-propoxy-1-naphthol, 2-[p-(1', 5'-Dihydroxyphenethyl)-phenylazo]-4-acetamido-1-naphthol, 2-[p-(2', 5'-Dihydroxyphenethyl)-phenylazo]-4-methoxy-1-naphthol, 2-[p-(2', 5'-Dihydroxyphenethyl)-phenylazo]-4-ethoxy-1-naphthol, 1-[p-(2', 5'-Dihydroxyphenethyl)-phenylazo]-4-n-propyl-1-naphthol.



2-[p-(2', 5'-Dihydroxyphenethyl)-phenylazo]-4-[1'', 4''-dioxahexyl]-1-naphthol, 1,4-bis[ $\beta$ -(2', 5'-Dihydroxyphenyl)-ethylamino]

5 anthraquinone, 1-Chloro-4-[ $\beta$ -(2', 5'-dihydroxyphenyl)-ethylamino]anthraquinone, N-Monobenzol-1,4-bis[ $\beta$ -(3', 4'-dihydroxyphenyl)ethylamino]-anthraquinone, N-Monobenzo-1,4-bis[ $\beta$ -(2', 5'-dihydroxyphenyl)-ethylamino]-anthraquinone, 5,8-Dihydroxy-1,4-bis[ $\beta$ -hydroquinonyl- $\alpha$ -methyl]-ethylamino]-anthraquinone,

10 1,4-bis(2', 5'-Dihydroxyaniline)anthraquinone, 1,5-bis(2',5'-Dihydroxyaniline)-4, 8-dihydroxy-anthaquinone,

15 1,4-bis[( $\beta$ -Hydroquinonyl- $\alpha$ -ethyl)ethylamino]-anthraquinone,

20 5-Hydroxy-1,4-bis[( $\beta$ -hydroquinonyl- $\alpha$ -methyl)-ethylamino]-anthraquinone, 1-( $\beta$ -Hydroxy- $\alpha$ -ethyl-ethylamino)-4-( $\beta$ -hydroquinonyl- $\alpha$ -methyl-ethylamino)-anthraquinone, 1-(Butanol-2'-amino)-5,8-dihydroxy-4-hydroquinonyl-iso-propylamino-anthaquinone.



1,4-bis[ $\beta$ -(2', 5'-Dihydroxyphenyl)-isopropylamino]-anthraquinone,





1-Acetoxy-2-{p-[ $\beta$ -(hydroquinonyl)-ethyl]-phenylazo}-4-methoxy-naphthalene,  
 1-Acetoxy-2-{p-[ $\beta$ -(hydroquinonyl)ethyl]-phenylazo}-4-[(2'-ethoxy)-ethoxy]-naphthalene,  
 1-Acetoxy-2-{p-[ $\beta$ -(hydroquinonyl)-ethyl]-phenylazo}-4-isopropoxynaphthalene,



- 30  $\alpha$ -[2-Methyl-5-hydroquinonylmethyl]-phenylazo]- $\beta$ -(2'-benzofuranyl)- $\beta$ -acetoxy-acrylonitrile,  $\alpha$ -[(2-Acetoxy-5-hydroquinonylmethyl)-phenylazo]- $\beta$ -(2'-furyl)- $\beta$ -acetoxy-acrylonitrile,  $\alpha$ -[(2-Acetoxy-5-hydroquinonyl-ethyl)-phenylazo]- $\beta$ -(2'-benzofuranyl)- $\beta$ -acetoxy-acrylonitrile,  $\alpha$ -[(2-Acetoxy-5-hydroquinonylmethyl)-phenylazo]- $\beta$ -(2'-5'-bromofuryl)- $\beta$ -acetoxy-acrylonitrile,  $\alpha$ -[(2-Acetoxy-5-hydroquinonylmethyl)-phenylazo]- $\beta$ -(2'-5'-methoxybenzofuranyl)- $\beta$ -acetoxy-acrylonitrile,  $\alpha$ -[(2-Acetoxy-5-hydroquinonylmethyl)-phenylazo]- $\beta$ -(2'-5'-bromobenzofuranyl)- $\beta$ -acetoxy-acrylonitrile,  $\alpha$ -[(2-Acetoxy-5-hydroquinonylmethyl)-phenylazo]- $\beta$ -(2'-3'-methylbenzofuranyl)- $\alpha$ -acetoxy-acrylonitrile, 45  $\beta$ -(2-Acetoxy-phenylazo)- $\beta$ -(2'-5'-hydroquinonylacetoamido-benzofuranyl)- $\beta$ -acetoxy-acrylonitrile,

1-Acetoxy-2-{p-[ $\beta$ -(hydroquinonyl)-ethyl]-phenylazo}-4-(1', 4'-dioxapentyl)-naphthalene,  $\alpha$ -50 [p-(2-Hydroquinonylethyl)-phenylazo]- $\beta$ -(2'-furyl)- $\beta$ -acetoxy-acrylonitrile,  $\alpha$ -[p-(2-Hydroquinonyl-ethyl)-phenylazo]- $\beta$ -(2'-benzofuranyl)- $\beta$ -acetoxy-acrylonitrile,  $\alpha$ -[m-(2-Hydroquinonylethyl)-phenylazo]- $\beta$ -(2'-benzofuranyl)- $\beta$ -acetoxy-acrylonitrile,  $\alpha$ -[p-(2-Hydroquinonylethyl)-phenylazo]- $\beta$ -(2'-5'-bromofuryl)- $\beta$ -acetoxy-acrylonitrile,  $\alpha$ -[p-(2-Hydroquinonylethyl)-phenylazo]- $\beta$ -(2'-5'-methoxy-benzofuranyl)- $\beta$ -acetoxy-acrylonitrile, 60  $\alpha$ -[p-(2-Hydroquinonylethyl)-phenylazo]- $\beta$ -(2'-5'-bromo-benzofuranyl)- $\beta$ -acetoxy-acrylonitrile,  $\alpha$ -[p-(2-Hydroquinonylethyl)-phenylazo]- $\beta$ -(2'-3'-methyl-benzofuranyl)- $\beta$ -acetoxy-acrylonitrile,  $\alpha$ -Phenylazo- $\beta$ -(2-(5'-hydroquinonylacetamido-benzofuranyl))- $\beta$ -acetoxy-acrylonitrile,  $\alpha$ -[p-(2-Hydroquinonylethyl)-phenylazo]- $\beta$ -(2'-benzofuranyl)- $\beta$ -methoxyacetoxy-acrylonitrile,



$\alpha$ -[(2-Acetoxy-5-hydroquinonylmethyl)phenylazo]- $\beta$ -(2'-benzofuranyl)- $\beta$ -acetoxy-acrylonitrile, 2-[m-(Hydroquinonyl-methyl)phenylazo]-3-

butyroyloxy-5-methyl-benzothiophene, 2-[[(2'-Chloro-5-hydroquinonylmethyl)phenylazo]-3-acetoxy-benzothiophene, 2-[p-(2'-Hydroquinonyl-ethyl)-phenylazo]-3-acetoxy-benzothiophene, 2-[p-(2'-Hydroquinonyl-ethyl)-phenylazo]-3-acetoxy-5-chloro-benzothiophene, 2-[(2'-Acetoxy-5'-hydroquinonylmethyl)-phenylazo]-3-acetoxy-benzothiophene, 2-[(2'-Methyl-5'-hydroquinonylmethyl)phenylazo]-3-acetoxy-benzothiophene,



2-[m-(Hydroquinonylmethyl)phenylazo]-3-acetoxybenzothiophene, 1,4-bis(2', 5'-Dihydroxyaniline)-9,10-dihydroxyanthracene, 1,5-bis(2',5'-Dihydroxyaniline)-4,8,9,10-tetrahydroxy-anthracene, 1,4-bis[ $\beta$ -(2',5'-Dihydroxyphenyl)-isopropylamino]-9,10-dihydroxyanthracene, 1,4-bis[ $\beta$ -(2', 5'-Dihydroxyphenyl)-ethylamino]-9,10-dihydroxyanthracene, 1-Chloro-4-[ $\beta$ -(2', 5'-dihydroxyphenyl)-ethylamino]-9,10-dihydroxyanthracene, 1,4-bis[ $\gamma$ -(2', 5'-Dihydroxyphenyl)-propylamino]-5,8,9,10-tetrahydroxyanthracene, 1-[ $\gamma$ -(2', 5'-Dihydroxyphenyl)propylamino]-4-( $\beta$ -hydroxyethylamino)-5,8,9,10-tetrahydroxyanthracene, 1-[ $\beta$ -Hydroquinonyl- $\alpha$ -methyl)ethylamino]-4-( $\beta$ -hydroxyethylamino)-5,8,9,10-tetrahydroxyanthracene, 1-[ $\beta$ -(2', 5'-Dihydroxyphenyl)-ethylamino]-5-( $\beta$ -hydroxyethylamino)-4,8,9,10-tetrahydroxyanthracene, 1-[ $\beta$ -(2', 5'-Dihydroxyphenyl)-ethylamino]-4-hexylamino-5,8,9,10-tetrahydroxyanthracene, 1,4-bis[( $\beta$ -Hydroquinonyl- $\alpha$ -ethyl)ethylamino]-5,8,9,10-tetrahydroxyanthracene, 1,4-bis[( $\beta$ -Hydroquinonyl- $\alpha$ -methyl)ethylamino]-5,8,9,10-tetrahydroxyanthracene, 1,4-bis[( $\beta$ -Hydroquinonyl- $\alpha$ -ethyl)ethylamino]-9,10-dihydroxyanthracene, 1,4-bis[( $\beta$ -Hydroquinonyl- $\alpha$ -methyl)-ethyl-amino]-5,9,10-trihydroxyanthracene, 1-( $\beta$ -Hydroxy- $\alpha$ -ethyl-ethylamino)-4-( $\beta$ -hydroquinonyl- $\alpha$ -methyl-ethylamino)-9,10-dihydroxyanthracene, 1-(Butanol-

Diamino-2-[ $\epsilon$ -( $\alpha$ -ethyl-2', 5'-dihydroxyhydrocinnamido)-penoxy]-9,10-dihydroxyanthracene, 1,4-Diamino-2-[ $\epsilon$ -(2',5'-dihydroxyhydrocinnamido)penoxy]-9,10-dihydroxyanthracene,



1,4-bis[( $\gamma$ -Hydroquinonyl- $\alpha$ -methyl)-propylamino]-5,8,9,10-tetrahydroxyanthracene, 1-(o-Carboxyphenyl)-3-phenyl-4-[p-(2', 5'-trifluoroacetoxy- $\beta$ -phenylethyl)phenylazo]-5-hydroxypyrazole lactone,



1-(o-Carboxyphenyl)-3-N-phenylcarbamoyl-4-[p-( $\beta$ -hydroquinonyl-ethyl)phenylazo]-5-hydroxypyrazole lactone,  $\alpha$ -{[2-butyroyloxy-5-(2', 5'-butyroyloxy-phenylmethyl)-pehnylazo]-2''-benzofuranyl}- $\beta$ -butyroyloxyacrylonitrile, 2-[m-(2',5'-Butyroyloxy-phenylmethyl)phenylazo]-3-butyroyloxybenzothiophene,  $\alpha$ -[p-(2,5-Butyroyloxy- $\beta$ -phenylethyl)-phenylazo]- $\beta$ -(2'-benzofuranyl)- $\beta$ -butyroyloxy-acethonitrile,



and

2'-amino)-4-( $\beta$ -hydroquinonyl-isopropylamino)-5,8,9,10-tetrahydroxyanthracene, 1,8-bis[( $\beta$ -Hydroquinonyl- $\alpha$ -methyl)ethylamino]-4,5,9,10-tetrahydroxyanthracene, N-Monobenzol-1,4-bis[ $\beta$ -(3', 4'-dihydroxyphenyl)-ethylamino]-9,10-dihydroxyanthracene, N-Monobenzol-1,4-bis[ $\beta$ -(2', 5'-dihydroxyphenyl)-ethylamino]-9,10-dihydroxyanthracene, 1,4-Diamino-2-[ $\epsilon$ -( $\alpha$ -methyl-2', 5'-dihydroxyhydrocinnamido)-penoxy]-9,10-dihydroxyanthracene, 1,4-

2-[p-(2',5'-Ethoxyxaloxophenethyl)phenylazo]-4-methoxy-1-naphthol.

18. The silver halide developing agent dispersion according to claim 5, wherein the auxiliary developing agent is selected from the group consisting of phenylhydroquinone, 2-hydroxyphenylhydroquinone, phenoxyhydroquinone, 4-methylphenylhydroquinone, 1,4-dihydroxynaphthalene, 2-(4-aminophenethyl)-5-bromohydroquinone, 2-(4-aminophenethyl)-5-methyl-

hydroquinone, 4-aminophenethylhydroquinone, 2,5-dimethoxyhydroquinone, 2,5-dibutoxyhydroquinone, m-xylohydroquinone, bromohydroquinone, 3,6-dichlorohydroquinone, 2-dimethylaminomethyltoluhydroquinone, 2-cyclohexylhydroquinone, sec-butylhydroquinone, 2,5-dichlorohydroquinone, 2,5-diisopropylhydroquinone, 2,5-diiodohydroquinone, 3-chlorotoluhydroquinone, tetrachlorohydroquinone, 2,5-diphenylhydroquinone, 2,5-diresorcylydroquinone, 2,5-dioctylhydroquinone, dodecylhydroquinone, 4-methoxycatechol, 4-isopropoxycatechol, 3-isopropylcatechol, 4-phenylcatechol, 3,6-dimethylcatechol and 1,2-dihydroxy-5,8-methano-5,6,7,9-tetrahydronaphthalene.

19. The silver halide developing agent dispersion according to claim 6, wherein the high boiling solvent has a boiling point above 150° C.

20. The silver halide developing agent dispersion according to claim 19, wherein the solution of the silver halide developing agent in a high boiling solvent is dispersed in the form of fine colloidal particles.

21. The silver halide developing agent dispersion according to claim 20, wherein the colloidal particles have a particle size of less than about 1 $\mu$ .

22. The silver halide developing agent dispersion according to claim 20, wherein the colloidal particles have a particle size of less than about 0.3 $\mu$ .

23. The silver halide developing agent dispersion according to claim 1, wherein the hydrophilic organic colloid is selected from the group consisting of phthalated gelatin, polyvinyl alcohol, polyvinyl pyrrolidone, polyacrylamide, sodium polyacrylate, polyvinyl-2-methyldiazole, acrylamide/1-vinyl-2-methyldiazole copolymers, acrylamide/imidazole copolymers, acrylamide/1-vinyl-2-methyldiazole/acrylic acid copolymers, nitrocarboxymethylcellulose, N-vinylpyrrolidone-acrylic acid copolymers, N-vinylpyrrolidone-acrylic acid-methylacrylate copolymers, vinylphthalimide-acrylic acid copolymers, cellulose acetate hydrogen phthalate, poly-N-methylmethacrylamide, dimethyl-aminoethylmethacrylateacrylic acid copolymers, dimethylamino-ethylmethacrylate-acrylic acid-butyl acrylate copolymers, N,N-diethylacrylamide-acrylamide copolymers, poly-N-methylacrylamide copolymers, N-methylacrylamide-N-hydroxymethylacrylamide copolymers, poly-N-ethylacrylamide, methylvinylketoneacrylamide copolymers and N-vinylpyrrolidone-methacrolein copolymers.

24. The silver halide developing agent dispersion according to claim 19, wherein the high boiling solvent is selected from the group consisting of phosphoric acid esters, phthalic acid esters, aliphatic dibasic acid esters, aliphatic monobasic acid esters, amides, imides, alcohols, ethers, ketones.

25. The silver halide developing agent dispersion according to claim 19, wherein the high boiling solvent is selected from the group consisting of triethyl phosphate, tri-n-butyl phosphate, triphenyl phosphate, tricresyl phosphate, tri-p-tertbutylphenyl phosphate, tri-2-ethylhexyl phosphate, methyl phthalate, ethyl phthalate, n-butyl phthalate, 2-ethylbutyl phthalate, n-propyl phthalate, n-amyl phthalate, isoamyl phthalate, n-octyl phthalate,  $\beta$ -methoxyethyl phthalate, ditetrahydrofurfuryl phthalate, ditetrahydrofurfuryladipate, n-octyladipate, 2-ethylhexyladipate, n-hexyladipate, 2-ethylbutyl-acetate, butylsebacate, ditetrahydrofurfurylsuccinate, dibutoxyethylsuccinate, oleic acid butyl es-

ter, oleic acid tetrahydrofurfuryl ester, o-methoxyphenyl acetate, stearic acid butyl ester, triethyl citrate, acetyltriethyl citrate, triethyleneglycol di-2-ethyl hexoate, acetylricinol acid methyl ester, acetylricinol acid methoxyethyl ester,  $\alpha$ -acetoxy-butylacetyl succinate, tetrahydrofurfuryl benzoate, diethyl lauryl amide, dibutyl lauryl amide, tetraethyl phthalamide, N-n-butyl acetanilide, N-methyl-p-methyl acetanilide, N-n-amyl succinimide, N-n-amyl phthalimide, lauloyl piperidine, 4-methyl-2-pentanol, furfuryl alcohol, methyl isobutyl carbinol, 2,4-di-n-amyl phenol, and the like; ethers such as ethyleneglycol monobenzyl ether; and ketones such as ethyl-N, N-di-n-butylcarbamate, 2-methyl cyclohexanone, 3-methyl cyclohexanone and 4-methyl cyclohexanone.

26. The silver halide developing agent dispersion according to claim 1, wherein the ratio of the silver halide developing agent to the hydrophilic organic colloid is in the range of about 2:1 to 1:2.

27. The silver halide developing agent dispersion according to claim 19, wherein the high boiling solvent is capable of easily dissolving the silver halide developing agent and is substantially water-insoluble.

28. The silver halide developing agent dispersion according to claim 27, wherein the solution of the silver halide developing agent further contains an oleophilic polymer.

29. The silver halide developing agent dispersion according to claim 28, wherein the oleophilic polymer is selected from the group consisting of polyvinyl acetate, polyvinyl butyral, polyvinyl chloride, polyvinyl propionate, polymethyl acrylate, polyethyl acrylate, polybutyl acrylate, polypropyl acrylate, polymethylmethacrylate, polyethylmethacrylate, polybutylmethacrylate and polypropylmethacrylate.

30. The silver halide developing agent dispersion according to claim 28, wherein the dispersion further contains a viscosity increasing agent.

31. The silver halide developing agent dispersion according to claim 30, wherein the viscosity increasing agent is selected from the group consisting of polyacrylamide, cellulose nitrate, and poly-p-sulfostyrene potassium salt.

32. The silver halide developing agent dispersion according to claim 2, wherein the amount of the surface active polymer ranges from about 0.5 to 50% by weight based on the silver halide developing agent.

33. The silver halide developing agent dispersion according to claim 2, wherein the silver halide developing agent comprises at least one dye developer.

34. The silver halide developing agent dispersion according to claim 2, wherein the silver halide developing agent comprises at least one dye developer and at least one auxiliary developing agent.

35. The silver halide developing agent dispersion according to claim 2, wherein a solution of the silver halide developing agent in a high boiling solvent is dispersed in an about 1 to 20% by weight aqueous solution of the hydrophilic organic colloid.

36. The silver halide developing agent dispersion according to claim 2, wherein the hydrophilic organic colloid is gelatin.

37. The silver halide developing agent dispersion according to claim 2, wherein the dispersion further contains an anionic or nonionic surface active agent.

38. The silver halide developing agent dispersion according to claim 37, wherein the surface active agent is selected from the group consisting of aliphatic acid

salts, alkylsulfates, alkylphosphates, alkylsulfonates, alkylarylsulfonates, formaldehyde-condensates with alkylnaphthalenesulfonates, alklydiphenyl-ether sulfonates, dialkylsulfosuccinates, polyoxyethylene, alkyl ethers and the sulfuric ester salts thereof, polyoxyethylene alkylaryl ethers and the sulfuric ester salts thereof, polyoxyethylene alkyl esters and the sulfuric ester salts thereof, sorbitan alkyl esters, polyoxyethylene sorbitan alkyl ester, polyoxyethylene mannitan monolauric acid ester and styrene-maleic acid half ester copolymer.

39. The silver halide developing agent dispersion according to claim 37, wherein the surface active agent is selected from the group consisting of sodium myristate, sodium palmitate, sodium stearate, sodium oleate, sodium linoleate, sodium laurate, sodium caprate, potassium laurate, potassium stearate, sodium octadecylsulfate, sodium decylsulfate, sodium dodecylsulfate, sodium tetradecylsulfate, sodium hexadecylsulfate, potassium decylsulfate, potassium oleylsulfate, sodium octylphosphate, sodium dioctylphosphate, sodium nonylphosphate, sodium decylphosphate, potassium undecylphosphate, potassium dodecylphosphate, potassium pentadecylphosphate, sodium dodecylsulfonate, sodium hexadecanesulfonate, sodium octadecanesulfonate, potassium octylbenzenesulfonate, sodium nonylbenzenesulfonate, sodium decylbenzenesulfonate, sodium undecylsulfonate, sodium dodecylbenzenesulfonate, sodium tridecylbenzenesulfonate, sodium dibutynaphthalenesulfonate, sodium decylnaphthalenesulfonate, sodium octylnaphthalenesulfonate, potassium pentylnaphthalenesulfonate, sodium formaldehyde-condensate with naphthalenesulfonate, sodium formaldehyde-condensate with butylnaphthalenesulfonate, sodium nonyldiphenylether sulfonate, sodium decyldiphenylether sulfonate, sodium dodecyldiphenylether disulfonate, sodium dihexylsulfosuccinate, sodium dioctylsulfosuccinate, sodium dinonylsulfosuccinate, polyoxyethylene lauryl ether, polyoxyethylene oleyl ether, sodium polyoxyethylene lauryl ether sulfate, sodium polyoxyethylene oleyl ether sulfate, polyoxyethylene dodecyl ether, polyoxyethylene tetradecyl ether, polyoxyethylene hexadecyl ether, polyoxyethylene octadecyl ether, sodium polyoxyethylene nonylphenyl ether sulfate, polyoxyethylene stearic acid ester, polyoxyethylene palmitic acid ester, sodium polyoxyethylene lauric acid ester sulfate, sodium polyoxyethylene capric acid ester sulfate, sodium polyoxyethylene myristic acid ester sulfate, sorbitan monostearic acid ester, sorbitan tristearic acid ester, sorbitan monooleic acid ester, sodium sorbitan trioleate, polyoxyethylene sorbitan monolauric acid ester, polyoxyethylene sorbitan monostearic acid ester, polyoxyethylene monooleic acid ester, polyoxyethylene sorbitan monopalmitic acid ester, polyoxyethylene trioleic acid ester, polyoxyethylene mannitan monolauric acid ester and styrenemaleic acid half ester copolymer.

40. The silver halide developing agent dispersion according to claim 33, wherein the dye developer is selected from the group consisting of 1-Phenyl-3-N-n-hexylcarbamoyl-4-p-(2-hydroquinonylethyl)-phenylazo-5-pyrazolone, 2-p-(2-Hydroquinonylethyl)-phenylazo-4-isopropoxy-1-naphthol, 1,4-bis[ $\beta$ -( $\beta$ -Hydroquinonyl-isopropyl)amino]-5,8-dihydroxy-anthraquinone, 1-Phenyl-3-n-butyl-carbamoyl-4-[p-

(2',5'-dihydroxyphenethyl)-phenylazo]-5-pyrazolone, 1-Phenyl-3-N-n-hexylcarbamoyl-4-[p-(2',5'-dihydroxyphenethyl)-phenylazo]-5-pyrazolone, 2-[p-(2',5'-Dihydroxyphenethyl)phenylazo]-4-isopropoxy-1-naphthol, 1-Phenyl-3-N-cyclohexylcarbamoyl-4-[p-(2',5'-dihydroxy-phenethyl)-phenylazo]-5-pyrazolone, 1-Phenyl-3-amido-4-[4'{p-2'',5''-dihydroxyphenethyl}-phenylazo]-2',5'-diethoxyphenylazo]-5-pyrazolone, 1-Phenyl-3-N-cyclohexylcarbamoyl-4-[p-(2',5'-dihydroxy-phenethyl)-phenylazo]-5-pyrazolone, 1-Phenyl-3-phenyl-4-[p-(2',5'-dihydroxyphenethyl)-phenylazo]-5-pyrazolone, 1-Phenyl-3-methyl-4-[p-1',5'-dihydroxyphenethyl)-phenylazo]-5-pyrazolone, 1-Phenyl-3-(N-n-heptyl)carbamoyl-4-[p-( $\beta$ -hydroquinonylethyl)-phenylazo]-5-pyrazolone, 1-(2'-Chlorophenyl)-3-(N-n-hexylcarbamoyl)-4-[p-( $\beta$ -hydroquinonylethyl)-phenylazo]-5-pyrazolone,



1-(2'-Methylphenyl)-3-(N-n-hexylcarbamoyl)-4-[p-( $\beta$ -hydroquinonylethyl)-phenylazo]-5-pyrazolone, 1-Acetoxy-2-[p-( $\beta$ -hydroquinoneethyl)-phenylazo]-4-methoxy-naphthalene, 4-Isobutoxy-2-[p-( $\beta$ -hydroquinoneethyl)-phenylazo]-1-naphthol, 2-{4'-[p-(2'',5''-Dihydroxyphenethyl)-phenylazo]- $\alpha$ -naphthyl-azo}-4-methoxy-1-naphthol, 2-[p-(2',5'-Dihydroxy-4'-methylphenethyl)-phenylazo]-4-propoxy-1-naphthol, 2-[p-(1',5'-Dihydroxyphenethyl)-phenylazo]-4-acetamido-1-naphthol, 2-[p-(2',5'-Dihydroxyphenethyl)-phenylazo]-4-methoxy-1-naphthol, 2-[p-(2',5'-Dihydroxyphenethyl)-phenylazo]-4-ethoxy-1-naphthol, 1-[p-(2',5'-Dihydroxyphenethyl)-phenylazo]-4-n-propyl-1-naphthol,



2-[p-(2',5'-Dihydroxyphenethyl)-phenylazo]-4-[1',4'',-dioxahexyl]-1-naphthol, 1,4-bis[ $\beta$ -(2',5'-Dihydroxyphenyl)-ethylamino]anthraquinone, 1-Chloro-4-[ $\beta$ -(2',5'-dihydroxyphenyl)-ethylamino]anthraquinone, N-Monobenzol-1,4-bis[ $\beta$ -(3',4'-dihydroxyphenyl)ethylamino]-anthraquinone, N-Monobenzol-1,4-bis[ $\beta$ -(2',5'-dihydroxyphenyl)-ethylamino]-anthraquinone, 5,8-Dihydroxy-1,4-bis[ $\beta$ -(hydroquinonyl- $\alpha$ -methyl)-ethylamino]-anthraquinone, 1,4-bis(2',5'-Dihydroxyaniline)anthraquinone,

35

1,5-bis(2',5'-Dihydroxyaniline)-4,8-dihydroxy-anthraquinone,  
 1,4-bis[( $\beta$ -Hydroquinonyl- $\alpha$ -ethyl)ethylamino]-anthraquinone,  
 5-Hydroxy-1,4-bis[( $\beta$ -hydroquinonyl- $\alpha$ -methyl)-ethylamino]-anthraquinone, 1-( $\beta$ -Hydroxy- $\alpha$ -ethyl-ethylamino)-4-( $\beta$ -hydroquinonyl- $\alpha$ -methyl-ethylamino)-anthraquinone, 1-(Butanol-2'-amino)-5,8-dihydroxy-4-hydroquinonyl-isopropylamino-anthraquinone,



1,4-bis[ $\beta$ -(2',5'-Dihydroxyphenyl)-isopropylamino]-anthraquinone,



36

1-Acetoxy-2-{p-[ $\beta$ -(hydroquinonyl)-ethyl]-phenylazo}-4-methoxy-naphthalene, 1-Acetoxy-2-{p-[ $\beta$ -(hydroquinonyl)ethyl]-phenylazo}-4-[2'-ethoxy-ethoxy]-naphthalene, 1-Acetoxy-2-{p-[ $\beta$ -(hydroquinonyl)-ethyl]-phenylazo}-4-isopropoxy-naphthalene,

5

10



15

1-Acetoxy-2-{p-[ $\beta$ -(hydroquinonyl)-ethyl]-phenylazo}-4-(1',4'-dioxapentyl)-naphthalene,  $\alpha$ -[p-(2-Hydroquinonyl-ethyl)-phenylazo]- $\beta$ -(2'-furyl)- $\beta$ -acetoxy-acrylonitrile,  $\alpha$ -[p-(2-Hydroquinonyl-ethyl)-phenylazo]- $\beta$ -(2'-benzofuranyl)- $\beta$ -acetoxy-acrylonitrile,  $\alpha$ -[m-(2-Hydroquinonyl-ethyl)-phenylazo]- $\beta$ -(2'-benzofuranyl)- $\beta$ -acetoxyacrylonitrile,  $\alpha$ -[p-(2-Hydroquinonyl-ethyl)-phenylazo]- $\beta$ -(2'-(5'-bromofuryl))- $\beta$ -acetoxy-acrylonitrile,  $\alpha$ -[p-(2-Hydroquinonyl-ethyl)-phenylazo]- $\beta$ -(2'-(5'-bromophenyl))- $\beta$ -acetoxy-acrylonitrile,

20

25

30



methoxy-benzofuranyl]) $\beta$ -acetoxy-acrylonitrile,  $\alpha$ -[p-(2-Hydroquinonyl-ethyl)-phenylazo]- $\beta$ -[2'-5'-bromo-benzofuranyl]- $\beta$ -acetoxy-acrylonitrile,  $\alpha$ -[p-(2-Hydroquinonyl-ethyl)-phenylazo]- $\beta$ -2'-3'-methyl-benzofuranyl]- $\beta$ -acetoxy-acrylonitrile,  $\alpha$ -Phenylazo- $\beta$ -[2-(5'-hydroquinonylacetamido-benzofuranyl)]- $\beta$ -acetoxy-acrylonitrile,  $\alpha$ -[p-(2-Hydroquinonyl-ethyl)-phenylazo]- $\beta$ -(2'-benzofuranyl)- $\beta$ -methoxyacetoxy-acrylonitrile,



$\alpha$ -[(2-Methyl-5-hydroquinonylmethyl)-phenylazo]- $\beta$ -(2'-benzofuranyl)- $\beta$ -acetoxy-acrylonitrile,  $\alpha$ -[(2-Acetoxy-5-hydroquinonylmethyl)-phenylazo]- $\beta$ -(2'-furyl)- $\beta$ -acetoxy-acrylonitrile,  $\alpha$ -[(2-Acetoxy-5-(2'-hydroquinonyl-ethyl))-phenylazo]- $\beta$ -(2'-benzofuranyl)- $\beta$ -acetoxy-acrylonitrile,  $\alpha$ -[(2-Acetoxy-5-hydroquinonylmethyl)-phenylazo]- $\beta$ -(2'-5'-bromofuryl)- $\beta$ -acetoxy-acrylonitrile,  $\alpha$ -[(2-Acetoxy-5-hydroquinonylmethyl)-phenylazo]- $\beta$ -(2'-5'-methoxybenzofuranyl)- $\beta$ -acetoxy-acrylonitrile,  $\alpha$ -[(2-Acetoxy-5-hydroquinonylmethyl)-phenylazo]- $\beta$ -(2'-5'-bromobenzofuranyl)- $\beta$ -acetoxy-acrylonitrile,  $\alpha$ -[(2-Acetoxy-5-hydroquinonylmethyl)-phenylazo]- $\beta$ -(2'-3'-methylbenzofuranyl)]- $\alpha$ -acetoxy-acrylonitrile,  $\beta$ -(2-Acetoxyphenylazo)- $\beta$ -(2'(5'-hydroquinonylacetamido-benzofuranyl)]- $\beta$ -acetoxyacrylonitrile,

2-[m-(Hydroquinonylmethyl)phenylazo]-3-acetoxybenzothiophene, 1,4-bis(2',5'-Dihydroxyaniline)-9,10-dihydroxyanthracene, 1,5-bis(2',5'-Dihydroxyaniline)-4,8,9,10-tetrahydroxy-anthracene, 1,4-bis[ $\beta$ -(2',5'-Dihydroxyphenyl)-isopropylamino]-9,10-dihydroxyanthracene, 1,4-bis[ $\beta$ -(2',5'-Dihydroxyphenyl)-ethylamino]-9,10-dihydroxyanthracene, 1-Chloro-4-[ $\beta$ -(2',5'-dihydroxyphenyl)-ethylamino]-9,10-dihydroxyanthracene, 1,4-bis[ $\gamma$ -(2',5'-Dihydroxyphenyl)-propylamino]-5,8,9,10-tetrahydroxyanthracene, 1-[ $\gamma$ -(2',5'-Dihydroxyphenyl)-propylamino]-4-( $\beta$ -hydroxyethylamino)-5,8,9,10-tetrahydroxyanthracene, 1-[ $\beta$ -(2',5'-Dihydroxyphenyl)-ethylamino]-4-( $\beta$ -hydroxyethylamino)-5,8,9,10-tetrahydroxyanthracene, 1-[ $\beta$ -(2',5'-Dihydroxyphenyl)-ethylamino]-5-( $\beta$ -hydroxyethylamino)-



$\alpha$ -[(2-Acetoxy-5-hydroquinonylmethyl)phenylazo]- $\beta$ -(2'-benzofuranyl)- $\beta$ -acetoxy-acrylonitrile, 2-[m-(Hydroquinonylmethyl)phenylazo]-3-butyroyloxy-5-methyl-benzothiophene, 2-[(2'-Chloro-5-hydroquinonylmethyl)phenylazo]-3-acetoxy-benzothiophene, 2-[p-(2'-Hydroquinonyl-ethyl)-phenylazo]-3-acetoxy-benzo-thiophene, 2-[p-(2'-Hydroquinonyl-ethyl)phenylazo]-3-acetoxy-5-chloro-benzothiophene, 2-[(2'-Acetoxy-5-hydroquinonylmethyl)phenylazo]-3-acetoxy-benzothiophene, 2-[(2'-Methyl-5'-hydroquinonylmethyl)phenylazo]-3-acetoxybenzothiophene,

4,8,9,10-tetrahydroxyanthracene, 1,5-bis[( $\beta$ -Hydroquinonyl- $\alpha$ -methyl)-ethylamino]-4,8,9,10-tetrahydroxyanthracene, 1-[ $\beta$ -(2',5'-Dihydroxyphenyl)ethylamino]-4-hexylamino-5,8,9,10-tetrahydroxyanthracene, 1,4-bis[( $\beta$ -Hydroquinonyl- $\alpha$ -ethyl)ethylamino]-5,8,9,10-tetrahydroxyanthracene, 1,4-bis[( $\beta$ -Hydroquinonyl- $\alpha$ -methyl)ethylamino]-5,8,9,10-tetrahydroxyanthracene, 1,4-bis[( $\beta$ -Hydroquinonyl- $\alpha$ -ethyl)ethylamino]-9,10-dihydroxyanthracene, 1,4-bis[( $\beta$ -Hydroquinonyl- $\alpha$ -methyl)-ethylamino]-5,9,10-trihydroxyanthracene, 1-( $\beta$ -Hydroxy- $\alpha$ -ethyl-ethylamino)-4-( $\beta$



39

hydroquinonyl- $\alpha$ -methyl-ethylamino)-9,10-dihydroxyanthracene, 1-(Butanol-2'-amino)-4-( $\beta$ -hydroquinonyl-isopropylamino)-5,8,9,10-tetrahydroxyanthracene, 1,8-bis[( $\beta$ -Hydroquinonyl- $\alpha$ -methyl)ethylamino]-4,5,9,10-tetrahydroxyanthracene, N-Monobenzol-1,4-bis[ $\beta$ -(3',4'-dihydroxyphenyl)-ethylamino]-9,10-dihydroxyanthracene, N-Monobenzol-1,4-bis[ $\beta$ -(2',5'-dihydroxyphenyl)-ethylamino]-9,10-dihydroxyanthracene, 1,4-Diamino-2-[ $\epsilon$ -( $\alpha$ -methyl-2',5'-dihydroxyhydrocinnamido)-pentox]-9,10-dihydroxyanthracene, 1,4-Diamino-2-[ $\epsilon$ ( $\alpha$ -ethyl-2',5'-dihydroxyhydrocinnamido)-pentox]-9,10-dihydroxyanthracene, 1,4-Diamino-2-[ $\epsilon$ -(2',5'-dihydroxyhydrocinnamido)-pentox]-9,10-dihydroxyanthracene,



1,4-bis[( $\gamma$ -Hydroquinonyl- $\alpha$ -methyl)-propylamino]-5,8,9,10-tetrahydroxyanthracene, 1-(o-Carboxyphenyl)-3-phenyl-4-[p-(2',5'-trifluoroacetoxy- $\beta$ -phenylethyl)phenylazo]-5-hydroxypyrazole lactone,



1-(o-Carboxyphenyl)-3-N-phenylcarbamoyl-4-[p-( $\beta$ -hydroquinonylethyl)phenylazo]-5-hydroxypyrazole lactone,  
 $\alpha$ -[(2-Butyroyloxy-5-(2',5'-butyroyloxy-phenylmethyl)]-phenylazo)-2'-benzofuranyl]- $\beta$ -butyroyloxyacrylonitrile, 2-[m-(2',5'-Butyroyloxyphenylmethyl)phenylazo]-3-butyroyloxybenzothiophene,  $\alpha$ -[p-(2,5-Butyroyloxy- $\beta$ -phenylethyl)-phenylazo]- $\beta$ -(2'-benzofuranyl)- $\beta$ -butyroyloxy-acetonitrile,



40

2-[p-(2',5'-Ethoxyoxaloxyphenethyl)phenylazo]-4-methoxy-1-naphthol.

41. The silver halide developing agent dispersion according to claim 34, wherein the auxiliary developing agent is selected from the group consisting of phenylhydroquinone, 2-hydroxyphenylhydroquinone, phenoxhydroquinone, 4-methylphenyl-hydroquinone, 1,4-dihydroxynaphthalene, 2-(4-aminophenethyl)-5-bromohydroquinone, 2-(4-aminophenethyl)-5-methylhydroquinone, 4-aminophenethylhydroquinone, 2,5-dimethoxyhydroquinone, 2,5-dibutoxyhydroquinone, m-xylohydroquinone, bromohydroquinone, 3,6-dichlorohydroquinone, 2-dimethylaminomethyltoluhydroquinone, 2-cyclohexylhydroquinone, sec-butylhydroquinone, 2,5-dichlorohydroquinone, 2,5-diisopropylhydroquinone, 2,5-diiodohydroquinone, 3-chlorotoluhydroquinone, tetrachlorohydroquinone, 2,5-diphenylhydroquinone, 2,5-diresorcylydroquinone, 2,5-diocetylhydroquinone, dodecylhydroquinone, 4-methoxycatechol, 4-isopropoxycatechol, 3-isopropylcatechol, 4-phenylcatechol, 3,6-dimethylcatechol and 1,2-dihydroxy-5,8-methano-5,6,7,9-tetrahydronaphthalene.

42. The silver halide developing agent dispersion according to claim 35, wherein the high boiling solvent has a boiling point above 150°C.

43. The silver halide developing agent dispersion according to claim 42, wherein the solution of the silver halide developing agent in a high boiling solvent is dispersed in the form of fine colloidal particles.

44. The silver halide developing agent dispersion according to claim 43, wherein the colloidal particles have a particle size of less than about 1 $\mu$ .

45. The silver halide developing agent dispersion according to claim 43, wherein the colloidal particles have a particle size of less than about 0.3 $\mu$ .

46. The silver halide developing agent dispersion according to claim 2, wherein the hydrophilic organic colloid is selected from the group consisting of phthalated gelatin, polyvinyl alcohol, polyvinyl pyrrolidone, polyacrylamide, sodium polyacrylate, polyvinyl-2-methylidazole, acrylamide/1-vinyl-2-methylimidazole copolymers, acrylamide/imidazole copolymers, acrylamide/1-vinyl-2-methylimidazole/acrylic acid copolymers, nitrocarboxymethylcellulose, N-vinylpyrrolidone-acrylic acid copolymers, N-vinylpyrrolidone-acrylic acid-methylacrylate copolymers, vinylphthalimide-acrylic acid copolymers, cellulose acetate hydrogen phthalate, poly-N-methylmethacrylamide, dimethyl-aminoethylmethacrylateacrylic acid copolymers, dimethylamino-ethylmethacrylate-acrylic acid-butyl acrylate copolymers, N,N-diethylacrylamide-acrylamide copolymers, poly-N-methylacrylamide copolymers, N-methylacrylamide-N-hydroxymethylacrylamide copolymers, poly-N-ethylacrylamide, methylvinylketoneacrylamide copolymers and N-vinylpyrrolidone-methacrolein copolymers.

41

47. The silver halide developing agent dispersion according to claim 42, wherein the high boiling solvent is selected from the group consisting of phosphoric acid esters, phthalic acid esters, aliphatic dibasic acid esters, aliphatic monobasic acid esters, amides, imides, alcohols, ethers, ketones.

48. The silver halide developing agent dispersion according to claim 42, wherein the high boiling solvent is selected from the group consisting of triethyl phosphate, tri-n-butyl phosphate, triphenyl phosphate, tricresyl phosphate, tri-p-tertbutylphenyl phosphate, tri-2-ethylhexyl phosphate, methyl phthalate, ethyl phthalate, n-butyl phthalate, 2-ethylbutyl phthalate, n-propyl phthalate, n-amyl phthalate, isoamyl phthalate, n-octyl phthalate,  $\beta$ -methoxyethyl phthalate, ditetrahydrofurfuryl phthalate, ditetrahydrofurfuryladipate, n-octyladipate, 2-ethylhexyladipate, n-hexyladipate, 2-ethylbutyl-acetate, butylsebacate, ditetrahydrofurfurylsuccinate, dibutoxyethylsuccinate, oleic acid butyl ester, oleic acid tetrahydrofurfuryl ester, o-methoxyphenyl acetate, stearic acid butyl ester, triethyl citrate, acetyltriethyl citrate, triethyleneglycol di-2-ethyl hexoate, acetylricinol acid methyl ester, acetylricinol acid methoxyethyl ester,  $\alpha$ -acetoxy-butylacetyl succinate, tetrahydrofurfuryl benzoate, diethyl lauryl amide, dibutyl lauryl amide, tetraethyl phthalamide, N-n-butyl acetanilide, N-methyl-p-methyl acetanilide, N-n-amyl succinimide, N-n-amyl phthalimide, lauloyl piperidine, 4-methyl-2-pentanol, furfuryl alcohol, methyl isobutyl carbinol, 2,4,-di-n-amyl phenol, and the like; ethers such as ethyleneglycol monobenzyl ether; and ketones

42

such as ethyl-N, N-di-n-butylcarbamate, 2-methyl cyclohexanone, 3-methyl cyclohexanone and 4-methyl cyclohexanone.

49. The silver halide developing agent dispersion according to claim 2, wherein the ratio of the silver halide developing agent to the hydrophilic organic colloid is in the range of about 2:1 to 1:2.

50. The silver halide developing agent dispersion according to claim 42, wherein the high boiling solvent is capable of easily dissolving the silver halide developing agent and is substantially water-insoluble.

51. The silver halide developing agent dispersion according to claim 50, wherein the solution of the silver halide developing agent further contains an oleophilic polymer.

52. The silver halide developing agent dispersion according to claim 51, wherein the oleophilic polymer is selected from the group consisting of polyvinyl acetate, polyvinyl butyral, polyvinyl chloride, polyvinyl propionate, polymethyl acrylate, polyethyl acrylate, polybutyl acrylate, polypropyl acrylate, polymethylmethacrylate, polyethylmethacrylate, polybutylmethacrylate and polypropylmethacrylate.

53. The silver halide developing agent dispersion according to claim 51, wherein the dispersion further contains a viscosity increasing agent.

54. The silver halide developing agent dispersion according to claim 53, wherein the viscosity increasing agent is selected from the group consisting of polyacrylamide, cellulose nitrate, and poly-p-sulfostyrene potassium salt.

\* \* \* \* \*

35

40

45

50

55

60

65